# EUROPEAN PATENT APPLICATION

(11) **EP 4 216 242 A1**
(43) Date of publication of application: **26.07.2023**
(21) Application number: 21869392.7
(22) Date of filing: 15.09.2021
(51) Int. Cl.: H01F 17/04, H01F 1/28

(54) **COMPOSITION, MAGNETIC-PARTICLE-CONTAINING FILM, AND ELECTRONIC COMPONENT**

(30) Priority: 18.09.2020 JP 2020157451
(71) Applicant: FUJIFILM Corporation, Tokyo 106-8620 (JP)
(72) Inventor: ISHIKAWA, Tatsuo, Haibara-gun, Shizuoka 421-0396 (JP); MIYATA, Tetsushi, Haibara-gun, Shizuoka 421-0396 (JP)
(74) Representative: HGF
(86) International application number: PCT/JP2021/033938
(87) International publication number: WO 2022/059706

(57) **Abstract**

An object of the present invention is to provide a composition that can form a magnetic particle-containing film having excellent magnetic permeability and excellent acid resistance, and has excellent sedimentation stability. Another object of the present invention is to provide a magnetic particle-containing film that relates to the composition, and an electronic component that includes the magnetic particle-containing film.

The composition according to an embodiment of the present invention contains magnetic particles that contain 70% to 90% by mass of Fe atoms and have a crystal structure of Fe, an average particle diameter of 2 to 30 µm, and an aspect ratio less than 8, and a rheology control agent.

## Description

### BACKGROUND OF THE INVENTION

### 1. Field of the Invention

The present invention relates to a composition, a magnetic particle-containing film, and an electronic component.

### 2. Description of the Related Art

With the performance upgrade and further miniaturization of electronic devices, the degree of integration of electronic circuits is increasing. As one of the materials for improving the degree of integration, there is a coating-type composition containing magnetic particles. Using such a composition enables a magnetic material to be mounted in any shape, which makes it easier to achieve miniaturization and performance upgrade of electronic devices compared to the conventional method of arranging individual pieces of magnetic materials on a chip.

Incidentally, the coating-type composition containing magnetic particles and a film formed of such a composition are exposed to an electronic circuit manufacturing process. Therefore, the composition and the film are required to have various types of durability.

For example, JP2019-067960A discloses "an inductor substrate manufacturing method including, in the following order, (A) step of laminating a resin sheet with a support which includes a support and a resin composition layer provided on the support on an inner layer substrate such that the resin composition layer is bonded to the inner layer substrate,
(B) step of thermally curing the resin composition layer to form an insulating layer,
(C) step of performing drilling on the insulating layer,
(D) step of performing a wet desmear treatment on a surface of the insulating layer by using an oxidant solution, and
(E) step of forming a conductor layer on the surface of the insulating layer that has undergone the wet desmear treatment,
in which an inductor is formed of a plurality of insulating layers and a plurality of conductor layers,
the resin composition layer is formed of a resin composition containing a magnetic filler, and
a weight loss rate of the magnetic filler is 0% or more and 40% or less in a case where the inductor substrate is stored at 20°C for 3 hours in an acidic solution having a pH of 1 (See claim 1). In JP2019-067960A, specifically, the magnetic filler (hereinafter, also called "coated magnetic particles") having magnetic powder and a coating layer which coats the magnetic powder is used to suppress "reduction in peel strength between an insulating layer and a conductor layer" that can occur in the step of performing a wet desmear treatment by using an oxidant solution.

### SUMMARY OF THE INVENTION

With reference to Examples of JP2019-067960A, the inventors of the present invention prepared and examined coated magnetic particles and a composition containing coated magnetic particles. As a result, the inventors have revealed that sometimes the acid resistance of a film formed of the composition does not reach the currently required level. Furthermore, the inventors have revealed that sometimes the coating layer is peeled off from the magnetic powder as the coated magnetic particles keep dispersing during the dispersion treatment of the coated magnetic particles.

By the way, a magnetic film is required to have excellent magnetic permeability as a basic performance. Furthermore, for a coating-type composition containing magnetic particles, as a basic performance, it is required the magnetic particles be excellently stably dispersed in the composition even after a long lapse of time (hereinafter, the performance will be also called "sedimentation stability").

An object of the present invention is to provide a composition that can form a magnetic particle-containing film having excellent magnetic permeability and excellent acid resistance and has excellent sedimentation stability. Another object of the present invention is to provide a magnetic particle-containing film that relates to the composition, and an electronic component that includes the magnetic particle-containing film.

The inventors of the present invention have found that the above objects can be achieved by the following constitution.
[1] A composition containing magnetic particles that contain 70% to 90% by mass of Fe atoms, have a crystal structure of Fe, an average particle diameter of 2 to 30 µm, and an aspect ratio less than 8, and
   a rheology control agent.
[2] A composition containing magnetic particles that contain 70% to 90% by mass of Fe atoms, have a diffraction peak which has a half-width of 0.2° to 3° and appears at 2θ in a range of 42° to 48° in an X-ray diffraction pattern obtained by X-ray diffraction analysis, have an average particle diameter of 2 to 30 µm, and have an aspect ratio less than 8, and
   a rheology control agent.
[3] The composition described in [1], in which the magnetic particles have a diffraction peak which has a half-width of 0.2° to 3° and appears at 2θ in a range of 42° to 48° in an X-ray diffraction pattern obtained by X-ray diffraction analysis.
[4] The composition described in any one of [1] to [3], in which a content of the magnetic particles is 70% to 90% by mass with respect to a total mass of the composition.
[5] The composition described in any one of [1] to [4], in which the rheology control agent is one or more substances selected from the group consisting of a polycarboxylic acid, a polycarboxylic anhydride, and an amide wax.
[6] The composition according to any one of [1] to [5], further containing a curable component that is cured by light or heat.
[7] The composition described in [6], in which the curable component includes a polymerizable compound.
[8] The composition described in [7], in which the polymerizable compound includes a compound that contains one or more epoxy groups and one or more oxetanyl groups.
[9] The composition described in any one of [1] to [8], further containing a polymerization initiator.
[10] The composition described in any one of [1] to [9], in which the composition substantially does not contain a solvent, or
   the composition further contains a solvent, and a content of the solvent is 1% by mass or more and less than 12% by mass with respect to a total mass of the composition.
[11] A magnetic particle-containing film formed of the composition described in any one of [1] to [10].
[12] An electronic component including the magnetic particle-containing film described in [11].
[13] The electronic component described in [12], in which the electronic component is used as an inductor.
[14] The electronic component described in [12], in which the electronic component is used as an antenna.

According to an aspect of the present invention, it is possible to provide a composition that can form a magnetic particle-containing film having excellent magnetic permeability and excellent acid resistance and has excellent sedimentation stability. Furthermore, according to an aspect of the present invention, it is possible to provide a magnetic particle-containing film that relates to the composition and an electronic component that includes the magnetic particle-containing film.

### DESCRIPTION OF THE PREFERRED EMBODIMENTS

Hereinafter, the present invention will be specifically described.

The following constituents will be described based on typical embodiments of the present invention in some cases. However, the present invention is not limited to the embodiments.

Regarding the notation of a group (atomic group) in the present specification, unless the gist of the present invention is missed, the notation without the terms "substituted" and "unsubstituted" includes both the group having no substituent and the group having a substituent. For example, "alkyl group" includes not only an alkyl group having no substituent (unsubstituted alkyl group) but also an alkyl group having a substituent (substituted alkyl group). Furthermore, in the present specification, "organic group" refers to a group having at least one carbon atom.

In the present specification, "actinic ray" or "radiation" means, for example, a bright line spectrum of a mercury lamp, a far ultraviolet ray represented by an excimer laser, extreme ultraviolet (EUV light), an X-ray, an electron beam (EB), and the like. In the present specification, "light" means an actinic ray or radiation.

Unless otherwise specified, "exposure" in the present specification means not only the exposure performed using a bright line spectrum of a mercury lamp, a far ultraviolet ray represented by an excimer laser, extreme ultraviolet, an X-ray, EUV light, and the like, but also the drawing performed using particle beams such as an electron beam and an ion beam.

In the present specification, a range described using "to" includes the numerical values listed before and after "to" as a lower limit and an upper limit.

In the present specification, (meth)acrylate represents acrylate and methacrylate, (meth)acryl represents acryl and methacryl, and (meth)acryloyl represents acryloyl and methacryloyl.

In the present specification, "solid content" of a composition means components forming a magnetic particle-containing film. In a case where the composition contains a solvent (such as an organic solvent or water), "solid content" means all components except for the solvent. In addition, a liquid component is also regarded as a solid content as long as this component forms the magnetic particle-containing film.

In the present specification, a weight-average molecular weight (Mw) is a polystyrene-equivalent value obtained by a Gel Permeation Chromatography (GPC) method.

The GPC method in the present specification is based on a method using HLC-8020GPC (manufactured by Tosoh Corporation), columns consisting of TSKgel SuperHZM-H, TSKgel SuperHZ4000, and TSKgel SuperHZ2000 (manufactured by Tosoh Corporation, 4.6 mm ID x 15 cm), and tetrahydrofuran (THF) as an eluent.

In the present specification, as each component, unless otherwise specified, one substance corresponding to each component may be used alone, or two or more substances corresponding to each component may be used in combination. Here, in a case where two or more substances are used in combination as each component, unless otherwise specified, the content of the component means the total content of the substances used in combination.

### [Composition]

The composition according to an embodiment of the present invention (hereinafter, sometimes also called "composition A") contains magnetic particles (hereinafter, also called "specific magnetic particles") that contain 70% to 90% by mass of Fe atoms and have a crystal structure of Fe (hereinafter, sometimes simply described as "crystal structure"), an average particle diameter of 2 to 30 µm, and an aspect ratio less than 8, and a rheology control agent.

Among the ferromagnetic metals, magnetic particles containing Fe atoms (hereinafter, also called "Fe atom-containing magnetic particles") exhibit high magnetic permeability. However, because the standard oxidation-reduction potential of the Fe atom-containing magnetic particles is quite negative (that is, the particles have strong ionization tendency), these particles are easily eluted into an acid in a case where the particles are immersed in an acidic liquid. That is, there is a concern that the magnetic particle-containing film containing the Fe atom-containing magnetic particles may have poor acid resistance though the film has excellent magnetic permeability. Presumably, the higher the content of the Fe atom-containing magnetic particles in the magnetic particles, the higher the magnetic permeability of the formed magnetic particle-containing film, and the more likely it is that the film will be dissolved in an acid, which may deteriorate the acid resistance. On this issue, the inventors of the present invention conducted studies. As a result, the inventors have revealed that in a case where the Fe atom-containing magnetic particles have a crystal structure, the acid resistance of the formed magnetic particle-containing film is markedly improved (as the reason, presumably, in a case where the Fe atom-containing magnetic particles has a crystal structure, even though the particles are immersed in an acidic liquid, the particles are unlikely to be oxidized, and the original composition thereof is unlikely to change, which may suppress the deterioration of magnetic permeability and result in excellent acid resistance). Particularly, the inventors have found that in a case where the Fe atom-containing magnetic particles have a crystal structure and have an Fe atom content of 70% to 90% by mass, the formed magnetic particle-containing film can achieve both the high magnetic permeability and excellent acid resistance. Based on the above findings, the inventors of the present invention further conducted studies. As a result, the inventors have revealed that the objects of the invention can be achieved by the constitution of the composition according to the embodiment of the present invention described above. The details of reason why the objects of the present invention can be achieved by the composition having such a constitution are unclear, but are roughly assumed to be as below.

As described above, by the constitution in which the specific magnetic particles have a crystal structure and a Fe atom content of 70% to 90% by mass, the formed magnetic particle-containing film can achieve both the high magnetic permeability and excellent acid resistance.

Furthermore, the specific magnetic particles having an aspect ratio less than 8 are likely to be isotropically arranged in the magnetic particle-containing film, which is assumed to contribute to the improvement of the magnetic permeability of the formed magnetic particle-containing film. On the other hand, the magnetic particles having an aspect ratio less than 8 are more likely to be deposited as sediments in the composition, compared to magnetic particles having an aspect ratio of 8 or more, which tends to negatively affect the sedimentation stability. Therefore, in the composition according to the embodiment of the present invention, the average particle diameter of the specific magnetic particles is set to 2 to 30 µm, and a rheology control agent is introduced into the composition, such that sedimentation stability is ensured. Presumably, introducing the rheology control agent into the composition may improve the dispersibility of the specific magnetic particles, which may allow the magnetic particles to be more uniformly arranged in the magnetic particle-containing film. It is considered that this may also contribute to the improvement of the magnetic permeability of the formed magnetic particle-containing film.

Hereinafter, further improving at least one or more properties among the sedimentation stability of the composition, the magnetic permeability of the formed magnetic particle-containing film, and the acid resistance of the formed magnetic particle-containing film will be also described as "further improving the effects of the present invention".

Hereinafter, first, various components contained in the composition will be described.

### [Magnetic particles]

### <Specific magnetic particles>

The composition contains specific magnetic particles.

The specific magnetic particles are magnetic particles that contain 70% to 90% by mass of Fe atoms and having a crystal structure of Fe, an average particle diameter of 2 to 30 µm, and an aspect ratio less than 8.

The specific magnetic particles contain iron atoms (Fe atoms) as metal atoms.

The iron atoms may be contained in the magnetic particles, as an alloy containing iron atoms (preferably a magnetic alloy containing iron atoms), an iron oxide (preferably a magnetic iron oxide), an iron nitride (preferably a magnetic iron nitride), or an iron carbide (preferably a magnetic iron carbide).

The content of the iron atoms is 70% to 90% by mass with respect to the total mass of the specific magnetic particles. In a case where the content of the iron atoms is 70% by mass or more with respect to the total mass of the specific magnetic particles, the formed magnetic particle-containing film has excellent magnetic permeability. In a case where the content of the iron atoms is 90% by mass or less with respect to the total mass of the specific magnetic particles, the formed magnetic particle-containing film has excellent acid resistance.

The lower limit of the content of the iron atoms with respect to the total mass of the specific magnetic particles is preferably 75% by mass or more, and more preferably 80% by mass or more. The upper limit of the content of the iron atoms is preferably 88% by mass or less with respect to the total mass of the specific magnetic particles.

The specific magnetic particles may contain other metal atoms different from the iron atoms.

"Other metal atoms" mentioned herein also include metalloid atoms such as boron, silicon, germanium, arsenic, antimony, and tellurium.

Those other metal atoms may be contained in the magnetic particles, as an alloy containing metal atoms (preferably a magnetic alloy), a metal oxide (preferably a magnetic oxide), a metal nitride (preferably a magnetic nitride), or a metal carbide (preferably a magnetic carbide).

In the specific magnetic particles, the lower limit of the content of the metal atoms (total content of the iron atoms and other metal atoms) with respect to the total mass of the specific magnetic particles is 70% by mass or more, preferably 75% by mass or more, and more preferably 80% by mass or more. In addition, the upper limit of the content of the metal atoms (iron atoms and other metal atoms) with respect to the total mass of the specific magnetic particles is preferably 100% by mass or less, and more preferably 90% by mass or less.

Examples of materials other than the iron atoms constituting the specific magnetic particles include Ni, Co, Al, Si, S, Sc, Ti, V, Cu, Y, Mo, Rh, Pd, Ag, Sn, Sb, Te, Ba, Ta, W, Re, Au, Bi, La, Ce, Pr, Nd, P, Zn, Sr, Zr, Mn, Cr, Nb, Pb, Ca, B, C, N, and O.

It is preferable that the specific magnetic particles contain, as materials other than the iron atoms, one or more atoms selected from the group consisting of Si, Cr, C, P, Cu, Nb, and B.

In a case where the specific magnetic particles contain Cu atoms, the content of the Cu atoms with respect to the total mass of the specific magnetic particles is preferably 0.1% to 10% by mass, more preferably 0.1% to 5% by mass, and even more preferably 0.1% to 3% by mass.

In a case where the specific magnetic particles contain Nb atoms, the content of the Nb atoms with respect to the total mass of the specific magnetic particles is preferably 2% to 10% by mass, more preferably 3% to 8% by mass, and even more preferably 4% to 6% by mass.

In a case where the specific magnetic particles contain B atoms, the content of the B atoms with respect to the total mass of the specific magnetic particles is preferably 1% to 4% by mass, and more preferably 2% to 4% by mass.

In a case where the specific magnetic particles contain Si atoms, the content of the Si atoms with respect to the total mass of the specific magnetic particles is preferably 1% to 20% by mass, more preferably 3% to 15% by mass, and even more preferably 5% to 10% by mass.

In a case where the specific magnetic particles contain Cr atoms, the content of the Cr atoms with respect to the total mass of the specific magnetic particles is preferably 0.001% to 1% by mass, more preferably 0.005% to 0.5% by mass, and even more preferably 0.01% to 0.1% by mass.

In a case where the specific magnetic particles contain C atoms, the content of the C atoms with respect to the total mass of the specific magnetic particles is preferably 0.001% to 1% by mass, more preferably 0.005% to 0.5% by mass, and even more preferably 0.01% to 0.2% by mass.

In a case where the specific magnetic particles contain P atoms, the content of the P atoms with respect to the total mass of the specific magnetic particles is preferably 0.001% to 10% by mass, more preferably 0.01% to 10% by mass, and even more preferably 0.1% to 10% by mass.

The content of each metal atoms in the specific magnetic particles can be identified by high-frequency inductively coupled plasma (ICP) emission spectroscopy.

The specific magnetic particles have a crystal structure of Fe (crystal structure).

The presence or absence of the crystal structure and the properties thereof can be identified by X-ray diffraction analysis, an electron microscope (for example, a transmission electron microscope (TEM)), or the like.

Examples of the type of crystal structure that the specific magnetic particles have include an α-Fe crystal phase. In a case where the specific magnetic particles have the aforementioned crystal structure, a peak can be observed at a diffraction angle (2θ) of, for example, 42° to 48° in an X-ray diffraction pattern obtained by the X-ray diffraction analysis by the 2θ method. In other words, in a case where the specific magnetic particles have the aforementioned crystal structure, in an X-ray diffraction pattern of the particles obtained by the X-ray diffraction analysis, the specific magnetic particles have a diffraction peak at 2θ in a range of 42° to 48°.

In the present specification, in a case where a diffraction peak appears at 2θ in a range of 42° to 48° in an X-ray diffraction pattern obtained by X-ray diffraction analysis, and a half-width of the diffraction peak is 5° or less, these properties are described as "have a crystal structure".

In the X-ray diffraction pattern, the half-width of the diffraction peak that appears at 2θ in a range of 42° to 48° is preferably 0.2° to 3°, more preferably 0.2° to 2°, and even more preferably 0.2° to 1°. The smaller the half-width of the diffraction peak, the denser the crystal structure, and the better the acid resistance of the formed magnetic particle-containing film.

The size of the crystal structure is, for example, 1 to 100 nm, and preferably 10 to 40 nm. "Size of a nano-crystal structure" mentioned herein corresponds to a perfect circle-equivalent diameter of a nano-crystal part (two-dimensionally observed region on a TEM image) confirmed in a case where the specific magnetic particles is observed with TEM.

In the specific magnetic particles, a portion other than the nano-crystal structure may be amorphous. That is, in the specific magnetic particles, the nano-crystal structure may be in the amorphous particles. The crystallization rate of the specific magnetic particles is not particularly limited, but is, for example, preferably 30% to 100% by volume, and more preferably 50% to 100% by volume.

The average particle diameter of the specific magnetic particles is a volume-based median diameter (D50), which is 2 to 30 µm. In a case where all the specific magnetic particles are divided into two parts by a threshold value which is a particle diameter at which the cumulative volume of the particles is 50%, the total volume of the specific magnetic particles having a large diameter equals to the total volume of the specific magnetic particles having a small diameter at a diameter which is the volume-based median diameter (D50) of the specific magnetic particles.

In a case where the average particle diameter (D50) of the specific magnetic particles is 2 µm or more, the magnetic permeability of the formed magnetic particle-containing film is excellent. On the other hand, in a case where the average particle diameter (D50) of the specific magnetic particles is 30 µm or less, the sedimentation stability of the specific magnetic particles in the composition is excellent.

In view of further improving the effects of the present invention, the upper limit of the average particle diameter (D50) of the specific magnetic particles is preferably 28 µm or less, and more preferably 25 µm or less.

The volume-based median diameter (D50) of the specific magnetic particles can be measured by a laser diffraction/scattering-type particle size distribution analyzer. As a measurement device, for example, a laser diffraction/scattering-type particle size distribution analyzer LA-960 (model number) manufactured by HORIBA, Ltd. can be used. However, the measurement device is not limited to this.

The aspect ratio of the specific magnetic particles is less than 8. In a case where the aspect ratio of the specific magnetic particles is less than 8, the sedimentation stability of the specific magnetic particles in the composition is excellent, and the magnetic permeability of the formed magnetic particle-containing film is excellent. In view of further improving the sedimentation stability of the specific magnetic particles in the composition, the aspect ratio of the specific magnetic particles is preferably less than 7, and more preferably 6 or less.

The lower limit of the aspect ratio of the specific magnetic particles is not particularly limited, but is preferably 1 or more.

In the present specification, the aspect ratio of particles is determined as follows. That is, the particles for which the aspect ratio is to be determined are observed with a transmission electron microscope (TEM), 200 particles are randomly extracted from the observed image, and the value of longest width A of each particle/shortest width B of each particle (A/B) is calculated for each of the 200 particles. The average of values of "A/B" calculated for the 200 particles is adopted as the aspect ratio of the particles.

The shape of the specific magnetic particles may be flat, elliptical, spherical, or amorphous, as long as the specific magnetic particles meet the requirements relating to the average particle diameter and aspect ratio described above.

The manufacturing method of the specific magnetic particles is not particularly limited.

Examples of one aspect of the manufacturing method of the specific magnetic particles include a manufacturing method of performing a heat treatment on Fe group-containing amorphous particles that contain 70% to 90% by mass of Fe atoms, an average particle diameter of 2 to 30 µm, and an aspect ratio less than 8. Specifically, the manufacturing method is a method of preparing Fe group-containing amorphous particles having the above composition first, and then performing a heat treatment on the amorphous particles at a high temperature (for example, at about 400°C to 600°C) to form a crystal structure in the amorphous particles.

Examples of another aspect of the manufacturing method of the specific magnetic particles include a manufacturing method of performing a heat treatment on Fe group-containing amorphous particles containing 70% to 90% by mass of Fe atoms to form a crystal structure in the amorphous particles, and then performing a predetermined dispersion treatment on the particles to adjust the average particle diameter and aspect ratio to a predetermined range. The procedure of the heat treatment is as described above.

As the specific magnetic particles, for example, it is also possible to use a commercially available product such as "KUAMET NC1" (manufactured by Epson Atmix Corporation).

The surface of each of the specific magnetic particles may be provided with a surface layer. In a case where the specific magnetic particles have a surface layer, it is possible to add functions to the specific magnetic particles according to the material of the surface layer.

Examples of the surface layer include an inorganic layer or an organic layer.

As a compound for forming an inorganic layer, in view of making it possible to form a surface layer excellent in at least one of the insulating properties, gas barrier properties, and chemical stability, a metal oxide, a metal nitride, a metal carbide, a phosphoric acid metal salt compound, a boric acid metal salt compound, or a silicic acid compound (for example, a silicic acid ester such as tetraethyl orthosilicate or a silicate such as sodium silicate) is preferable. Specific examples of elements contained in these compounds include Fe, Al, Ca, Mn, Zn, Mg, V, Cr, Y, Ba, Sr, Ge, Zr, Ti, Si, and rare earth elements.

Examples of the material constituting the inorganic layer obtained using the compound for forming an inorganic layer include silicon oxide, germanium oxide, titanium oxide, aluminum oxide, zirconium oxide, magnesium oxide, and the like. The inorganic layer may be a layer that contains two or more of these materials.

Examples of a compound for forming an organic layer include an acrylic monomer. Specific examples of the acrylic monomer include the compounds described in paragraphs "0022" and "0023" of JP2019-067960A.

Examples of the material constituting the organic layer obtained using the compound for forming an organic layer include an acrylic resin.

The thickness of the surface layer is not particularly limited. In view of enabling the surface layer to more effectively function, the thickness of the surface layer is preferably 3 to 1,000 nm.

In the composition, the content of the specific magnetic particles is preferably 70% to 90% by mass with respect to the total mass of the composition. Particularly, in view of further improving the magnetic permeability of the formed magnetic particle-containing film, the lower limit of the content of the specific magnetic particles is more preferably 75% by mass or more. In addition, in view of further improving coating suitability of the composition, the upper limit of the content of the specific magnetic particles is more preferably 85% by mass or less.

In the composition, the content of the specific magnetic particles is preferably 70% to 90% by mass with respect to the total solid content of the composition.

One kind of the specific magnetic particles may be used alone, or two or more kinds of the specific magnetic particles may be used in combination.

### [Rheology control agent]

The composition contains a rheology control agent.

The rheology control agent is a component that imparts thixotropy to the composition such that the composition exhibits high viscosity in a case where shearing force (shear rate) is low and exhibits low viscosity in a case where shearing force (shear rate) is high.

The content of the rheology control agent with respect to the total mass of the composition is preferably 0.1% to 35% by mass, more preferably 0.5% to 30% by mass, even more preferably 0.5% to 27% by mass, and particularly preferably 1% to 27% by mass.

The content of the rheology control agent with respect to the total solid content of the composition is preferably 0.1% to 35% by mass, more preferably 0.5% to 30% by mass, even more preferably 0.5% to 27% by mass, and particularly preferably 1% to 27% by mass.

Examples of the rheology control agent include an organic rheology control agent and an inorganic rheology control agent. Among these, an organic rheology control agent is preferable.

### <Organic rheology control agent>

The content of the organic rheology control agent with respect to the total mass of the composition is preferably 0.1% to 35% by mass, more preferably 0.5% to 30% by mass, even more preferably 0.5% to 25% by mass, and particularly preferably 1% to 25% by mass.

The content of the organic rheology control agent with respect to the total solid content of the composition is preferably 0.1% to 35% by mass, more preferably 0.5% to 30% by mass, even more preferably 0.5% to 25% by mass, and particularly preferably 1% to 25% by mass.

One organic rheology control agent may be used alone, or two or more organic rheology control agents may be used.

Examples of the organic rheology control agent include a compound that has one or more (preferably two or more) adsorptive groups and also has a steric repulsive structural group.

The adsorptive groups interact with the surface of the specific magnetic particles to make the organic rheology control agent adsorbed onto the surface of the specific magnetic particles.

Examples of the adsorptive groups include an acid group, a basic group, and an amide group.

Examples of the acid group include a carboxy group, a phosphoric acid group, a sulfo group, a phenolic hydroxyl group, and acid anhydride groups of these (such as an acid anhydride group of a carboxy group). In view of further improving the effects of the present invention, a carboxy group is preferable.

Examples of the basic group include an amino group (a group obtained by removing one hydrogen atom from ammonia, a primary amine, or a secondary amine) and an imino group.

As the adsorptive group, among these, a carboxy group or an amide group is preferable, and a carboxy group is more preferable.

Having a sterically bulky structure, the steric repulsive structural group introduces steric repulsion into the specific magnetic particles onto which the organic rheology control agent is adsorbed and maintains an appropriate space between the specific magnetic particles. As the steric repulsive structural group, for example, a chain-like group is preferable, a long-chain fatty acid group is more preferable, and a long-chain alkyl group is even more preferable.

The organic rheology control agent preferably has a hydrogen bonding unit.

The hydrogen bonding unit is a partial structure that functions to establish a hydrogen bonding network between the organic rheology control agents and between the organic rheology control agent and another component. The organic rheology control agent that contributes to the formation of the network may or may not be adsorbed onto the surface of the specific magnetic particles.

The hydrogen bonding unit may be the same as or different from the adsorptive group described above. In a case where the hydrogen bonding units are the same as the aforementioned adsorptive groups, some of the adsorptive groups are bonded to the surface of the specific magnetic particles and the others function as hydrogen bonding units.

As the hydrogen bonding units, carboxy groups or amide groups are preferable. Carboxy groups as the hydrogen bonding units are preferable because the carboxy groups readily take part in a curing reaction during the preparation of the magnetic particle-containing film. Amide groups as the hydrogen bonding units are preferable because the amide groups further improve the temporal stability of the composition.

In a case where the organic rheology control agent is a resin, the organic rheology control agent as a resin may have or substantially may not have a repeating unit having a graft chain that will be described later. In a case where the organic rheology control agent as a resin substantially does not have a repeating unit having a graft chain that will be described later, the content of the repeating unit having a graft chain that will be described later with respect to the total mass of the organic rheology control agent as a resin is preferably less than 2% by mass, more preferably 1% by mass or less, and even more preferably less than 0.1% by mass. The lower limit of the content of the repeating unit having a graft chain is 0% by mass or more.

The organic rheology control agent is preferably one or more substances selected from the group consisting of a polycarboxylic acid (compound having two or more carboxy groups), a polycarboxylic anhydride (compound having two or more acid anhydride groups consisting of carboxy groups), and an amide wax.

These may or may not be a resin.

In addition, these may correspond to an aggregation control agent and/or an anti-aggregation dispersant that will be described later.

Examples of organic rheology control agent include modified urea, a urea-modified polyamide, a fatty acid amide, polyurethane, a polyamide amide, a polymeric urea derivative, salts of these (such as carboxylates), and the like.

The modified urea is a reactant of an isocyanate monomer or an isocyanate monomer adduct and an organic amine. The modified urea is modified with a polyoxyalkylene polyol (such as polyoxyethylene polyol or polyoxypropylene polyol) and/or an alkyd chain, or the like. The urea-modified polyamide is, for example, a compound containing a urea bond and a compound obtained by introducing a medium-polarity group or a low-polarity group into the terminal of the compound containing a urea bond. Examples of the medium-polarity group or the low-polarity group include a polyoxyalkylene polyol (such as a polyoxyethylene polyol or polyoxypropylene polyol) and an alkyd chain. The fatty acid amide is a compound having a long-chain fatty acid group and an amide group in the molecule.

These may or may not be a resin.

In addition, these may correspond to an aggregation control agent and/or an anti-aggregation dispersant that will be described later.

The molecular weight of the organic rheology control agent (weight-average molecular weight in a case where the organic rheology control agent has a molecular weight distribution) is preferably in a range of 200 to 50,000.

In a case where the organic rheology control agent has an acid value, the acid value is preferably 5 to 400 mgKOH/g.

In a case where the organic rheology control agent has an amine value, the amine value is preferably 5 to 300 mgKOH/g.

### (Aggregation control agent)

Examples of the organic rheology control agent also include an aggregation control agent. The aggregation control agent may or may not be a resin.

The aggregation control agent has functions of being bonded to aggregates having a relatively high density, such as the specific magnetic particles, and dispersing optionally added other components (for example, a polymerizable compound and the like) in the composition such that bulky aggregates can be formed.

In a case where the composition contains an aggregation control agent, the specific magnetic particles in the composition are inhibited from forming a hard cake, and bulky aggregates are formed. Therefore, redispersibility can be improved.

Examples of the aggregation control agent include a cellulose derivative.

Examples of the cellulose derivative include carboxymethyl cellulose, methyl cellulose, hydroxyethyl cellulose, hydroxypropyl cellulose, hydroxypropyl methyl cellulose, hydroxypropyl ethyl cellulose, salts of these, and the like.

In a case where the composition contains an aggregation control agent, the content of the aggregation control agent with respect to the total mass of the composition is preferably 0.1% to 20% by mass, more preferably 0.3% to 15% by mass, and even more preferably 0.5% to 10% by mass.

The content of the aggregation control agent with respect to the total solid content of the composition is preferably 0.1% to 20% by mass, more preferably 0.3% to 15% by mass, and even more preferably 0.5% to 10% by mass.

### (Anti-aggregation dispersant)

Examples of the organic rheology control agent also include an anti-aggregation dispersant.

The anti-aggregation dispersant may or may not be a resin.

The anti-aggregation dispersant comprises a function of being adsorbed onto the surface of the specific magnetic particles such that the specific magnetic particles remain spaced apart from each other by at least a certain distance due to the interaction between the dispersants and that the specific magnetic particles are prevented from being directly aggregated with each other. As a result, the aggregation of the specific magnetic particles is suppressed, and even in a case where aggregates are formed, the density of the formed aggregates is relatively low. Furthermore, other components (for example, a polymerizable compound and the like) optionally added to the composition can be dispersed in the composition, and bulky aggregates can be formed. Therefore, redispersibility can be improved.

As the anti-aggregation dispersant, an alkylolammonium salt of a polybasic acid is preferable.

The polybasic acid may have two or more acid groups. Examples thereof include an acidic polymer containing a repeating unit having an acid group (for example, polyacrylic acid, polymethacrylic acid, polyvinyl sulfonic acid, polyphosphoric acid, and the like). Examples of polybasic acids other than the above include a polymer obtained by polymerizing an unsaturated fatty acid such as crotonic acid. The alkylolammonium salt of a polybasic acid is obtained by reacting these polybasic acids with alkylolammonium. The salt obtained by such a reaction usually contains the following partial structure.

-C(=O)-N(-R¹)(-R²-OH)

Here, R¹ is an alkyl group, and R² is an alkylene group.

The alkylolammonium salt of a polybasic acid is preferably a polymer containing a plurality of partial structures described above. In a case where the alkylolammonium salt of a polybasic acid is a polymer, the weight-average molecular weight thereof is preferably 1,000 to 100,000, and more preferably 5,000 to 20,000. The polymer of the alkylolammonium salt of a polybasic acid is bonded to the surface of the specific magnetic particles and forms a hydrogen bond with molecules of other anti-aggregation dispersants, such that the main chain structure of the polymer goes in between the specific magnetic particles and the specific magnetic particles are spaced apart from each other.

Examples of one of the suitable aspects of the anti-aggregation dispersant include amide wax which is a condensate formed by dehydrocondensation of (a) saturated aliphatic monocarboxylic acids and hydroxy group-containing aliphatic monocarboxylic acids, (b) at least any acids among polybasic acids, and (c) at least any amines among diamines and tetramines.

It is preferable that aforementioned (a) to (c) be used such that (a):(b):(c) = 1 to 3:0 to 5:1 to 6 in terms of molar ratio.

The saturated aliphatic monocarboxylic acids preferably have a carbon number of 12 to 22. Specific examples thereof include lauric acid, myristic acid, pentadecyl acid, palmitic acid, margaric acid, stearic acid, nonadecanoic acid, arachidic acid, behenic acid, and the like.

The hydroxy group-containing aliphatic monocarboxylic acids preferably have a carbon number of 12 to 22. Specific examples thereof include 12-hydroxystearic acid and dihydroxystearic acid.

Each of the saturated aliphatic monocarboxylic acids and each of the hydroxy group-containing aliphatic monocarboxylic acids may be used alone, or a plurality of saturated aliphatic monocarboxylic acids and a plurality of hydroxy group-containing aliphatic monocarboxylic acids may be used in combination.

The polybasic acids are preferably a carboxylic acid that has a carbon number of 2 to 12 and two or more replaceable hydrogen atoms, and more preferably a dicarboxylic acid. Examples of such a dicarboxylic acid include an aliphatic dicarboxylic acid such as oxalic acid, malonic acid, succinic acid, glutaric acid, adipic acid, pimelic acid, suberic acid, azelaic acid, sebacic acid, 1,10-decanedicarboxylic acid, or 1,12-dodecanedicarboxylic acid; an aromatic dicarboxylic acid such as phthalic acid, isophthalic acid, or terephthalic acid; and an alicyclic dicarboxylic acid such as 1,2-cyclohexanedicarboxylic acid, 1,3-cyclohexanedicarboxylic acid, 1,4-cyclohexanedicarboxylic acid, or cyclohexylsuccinic acid. Each of these polybasic acids may be used alone, or a plurality of these polybasic acids may be used in combination.

The diamines preferably have a carbon number of 2 to 14. Specifically, examples thereof include ethylenediamine, 1,3-propanediamine, 1,4-butanediamine, hexamethylenediamine, metaxylylenediamine, tolylenediamine, paraxylylenediamine, phenylenediamine, isophoronediamine, 1,10-decanediamine, 1,12-dodecanediamine, 4,4-diaminodicyclohexylmethane, and 4,4-diaminodiphenylmethane.

The tetramines preferably have a carbon number of 2 to 14. Specific examples thereof include butane-1,1,4,4-tetramine and pyrimidine-2,4,5,6-tetramine. Each of the diamines and each of the tetramines may be used alone, or a plurality of diamines and a plurality of tetramines may be used in combination.

The amount of diamines and tetramines is adjusted depending on the number of moles of the saturated aliphatic monocarboxylic acids or the hydroxy group-containing aliphatic monocarboxylic acids and the number of moles of the polybasic acids, such that the total number of carboxy groups is equivalent to the total number of amino groups. For example, in a case where the number of moles of an aliphatic dicarboxylic acid, which is polybasic acids, is n (n = 0 to 5) with respect to 2 moles of the aliphatic monocarboxylic acid, by setting the number of moles of diamines to (n + 1), the amount of acids is equivalent to the amount of amines.

This amide wax may be obtained as a mixture of a plurality of compounds having different molecular weights. The amide wax is preferably a compound represented by Chemical Formula (I). The amide wax may be a single compound or a mixture.

A-C-(B-C)ₘ-A··· (I)

In formula (I), A is a dehydroxylated residue of a saturated aliphatic monocarboxylic acid and/or a hydroxy group-containing saturated aliphatic monocarboxylic acid, B is a dehydroxylated residue of a polybasic acid, C is a dehydrogenated residue of a diamine and/or a tetramine, and m satisfies 0 ≤ m ≤ 5.

Examples of one of the suitable aspects of the anti-aggregation dispersant include a compound represented by the following Formula (II).

In Formula (II), R¹ represents a monovalent linear aliphatic hydrocarbon group with a carbon number of 10 to 25, R² and R³ each independently represent a divalent aliphatic hydrocarbon group with a carbon number of 2, 4, 6, or 8, a divalent alicyclic hydrocarbon group with a carbon number of 6, or a divalent aromatic hydrocarbon group, R⁴ represents a divalent aliphatic hydrocarbon group with a carbon number of 1 to 8, and R⁵ and R⁶ each independently represent a monovalent aliphatic hydrocarbon group with a carbon number of 1 to 3 or a hydroxyalkyl ether group.

In Formula (II), L¹ to L³ each independently represent an amide bond. In a case where L¹ and L³ each represent -CONH-, L² represents -NHCO-. In a case where L¹ and L³ each represent -NHCO-, L² represents -CONH-.

R¹ is a monovalent linear aliphatic hydrocarbon group with a carbon number of 10 to 25. Examples thereof include a linear alkyl group such as a decyl group, a lauryl group, a myristyl group, a pentadecyl group, a stearyl group, a palmityl group, a nonadecyl group, an eicosyl group, or a behenyl group; a linear alkenyl group such as a decenyl group, a pentadecenyl group, an oleyl group, or an eicosenyl group; and a linear alkynyl group such as a pentadecynyl group, an octadecynyl group, or a nonadecinyl group.

Particularly, R¹ is preferably a monovalent linear aliphatic hydrocarbon group with a carbon number of 14 to 25, and more preferably a monovalent linear aliphatic hydrocarbon group with a carbon number of 18 to 21. The linear aliphatic hydrocarbon group is preferably an alkyl group.

Examples of the divalent aliphatic hydrocarbon group with a carbon number of 2, 4, 6, or 8 represented by R² and R³ include an ethylene group, a n-butylene group, a n-hexylene group, and a n-octylene group.

Examples of the divalent alicyclic hydrocarbon group with a carbon number of 6 represented by R² and R³ include a 1,4-cyclohexylene group, a 1,3-cyclohexylene group, and a 1,2-cyclohexylene group.

Examples of the divalent aromatic hydrocarbon group represented by R² and R³ include an arylene group with a carbon number of 6 to 10, such as a 1,4-phenylene group, a 1,3-phenylene group, or a 1,2-phenylene group.

As R² and R³, among the above, in view of an excellent thickening effect, a divalent aliphatic hydrocarbon group with a carbon number of 2, 4, 6, or 8 is preferable, a divalent aliphatic hydrocarbon group with a carbon number of 2, 4, or 6 is more preferable, a divalent aliphatic hydrocarbon group with a carbon number of 2 or 4 is even more preferable, and a divalent aliphatic hydrocarbon group with a carbon number of 2 is still more preferable. The divalent aliphatic hydrocarbon group is preferably a linear alkylene group.

R⁴ represents a divalent aliphatic hydrocarbon group with a carbon number of 1 to 8. Among these, in view of an excellent thickening effect, a linear or branched alkylene group is preferable, and a linear alkylene group is more preferable.

The divalent aliphatic hydrocarbon group represented by R⁴ has a carbon number of 1 to 8. In view of an excellent thickening effect, the carbon number is preferably 1 to 7, more preferably 3 to 7, even more preferably 3 to 6, and particularly preferably 3 to 5.

Therefore, R⁴ is preferably a linear or branched alkylene group with a carbon number of 1 to 8, more preferably a linear alkylene group with a carbon number of 1 to 7, even more preferably a linear alkylene group with a carbon number of 3 to 7, particularly preferably a linear alkylene group with a carbon number of 3 to 6, and most preferably a linear alkylene group with a carbon number of 3 to 5.

Examples of the monovalent aliphatic hydrocarbon group with a carbon number of 1 to 3 represented by R⁵ and R⁶ include a linear or branched alkyl group with a carbon number of 1 to 3 such as a methyl group, an ethyl group, a propyl group, or an isopropyl group; a linear or branched alkenyl group with a carbon number of 2 or 3 such as a vinyl group, a 1-methylvinyl group, or a 2-propenyl group; a linear or branched alkynyl group with a carbon number of 2 or 3 such as an ethynyl group or a propynyl group.

Examples of the hydroxyalkyl ether group represented by R⁵ and R⁶ include a mono or di(hydroxy) C₁₋₃ alkyl ether group such as a 2-hydroxyethoxy group, a 2-hydroxypropoxy group, or a 2,3-dihydroxypropoxy group.

Especially, R⁵ and R⁶ preferably each independently represent a monovalent aliphatic hydrocarbon group with a carbon number of 1 to 3, more preferably each independently represent a linear or branched alkyl group with a carbon number of 1 to 3, even more preferably each independently represent a linear alkyl group with a carbon number of 1 to 3, and particularly preferably each independently represent a methyl group.

As the compound represented by Formula (II), the compounds represented by the following Formulas (II-1) to (II-9) are preferable.

Examples of the anti-aggregation dispersant include ANTI-TERRA-203, ANTI-TERRA-204, ANTI-TERRA-206, and ANTI-TERRA-250 (all are trade names, manufactured by BYK-Chemie GmbH.): ANTI-TERRA-U (trade name, manufactured by BYK-Chemie GmbH.): DISPER BYK-102, DISPER BYK-180, and DISPER BYK-191 (all are trade names, manufactured by BYK-Chemie GmbH.): BYK-P105 (trade name, manufactured by BYK-Chemie GmbH.): TEGO Disper 630 and TEGO Disper 700 (all are trade names, manufactured by Evonik Degussa Japan Co., Ltd.): Talen VA-705B (trade name, manufactured by KYOEISHA CHEMICAL CO., LTD.): FLOWNON RCM-300TL and FLOWNON RCM-230 AF (trade name, manufactured by KYOEISHA CHEMICAL CO., LTD., amide wax), and the like.

In a case where the composition contains an anti-aggregation dispersant, the content of the anti-aggregation dispersant with respect to the total mass of the composition is preferably 0.1% to 35% by mass, more preferably 0.3% to 30% by mass, and even more preferably 0.5% to 27% by mass.

The content of the anti-aggregation dispersant with respect to the total solid content of the composition is preferably 0.1% to 35% by mass, more preferably 0.3% to 30% by mass, and even more preferably 0.5% to 27% by mass.

### <Inorganic rheology control agent>

Examples of the inorganic rheology control agent include bentonite, silica, calcium carbonate, and smectite.

### [Other resins]

It is also preferable that the composition contain other resins.

The aforementioned other resins mean resins that do not correspond to rheology control agents that are resins.

The weight-average molecular weight of those other resins is preferably more than 2,000.

Examples of those other resins include a (meth)acrylic resin, an epoxy resin, an ene thiol resin, a polycarbonate resin, a polyether resin, a polyarylate resin, a polysulfone resin, a polyethersulfone resin, a polyphenylene resin, a polyarylene ether phosphine oxide resin, a polyimide resin, a polyamide imide resin, a polyolefin resin, a cyclic olefin resin, a polyester resin, a styrene resin, a phenoxy resin, and the like. One of these resins may be used alone, or two or more of these resins may be used by being mixed together. As the cyclic olefin resin, from the viewpoint of improving heat resistance, a norbornene resin is preferable. Examples of commercially available products of the norbornene resin include ARTON series manufactured by JSR Corporation (for example, ARTON F4520). Examples of the epoxy resin include an epoxy resin that is a glycidyl etherification product of a phenol compound, an epoxy resin that is a glycidyl etherification product of various novolac resins, an alicyclic epoxy resin, an aliphatic epoxy resin, a heterocyclic epoxy resin, a glycidyl ester-based epoxy resin, a glycidyl amine-based epoxy resin, an epoxy resin obtained by glycidylation of halogenated phenols, a condensate of a silicon compound having an epoxy group and another silicon compound, a copolymer of a polymerizable unsaturated compound having an epoxy group and another polymerizable unsaturated compound, and the like. As the epoxy resin, MARPROOF G-0150M, G-0105SA, G-0130SP, G-0250SP, G-1005S, G-1005SA, G-1010S, G-2050M, G-01100, and G-01758 (manufactured by NOF CORPORATION., epoxy group-containing polymers) and the like can also be used. In addition, as those other resins, the resins described in Examples of WO2016/088645A can also be used. In a case where those other resins have an ethylenically unsaturated group, particularly, a (meth)acryloyl group on a side chain, it is also preferable that the main chain and the ethylenically unsaturated group be bonded via a divalent linking group having an alicyclic structure.

Examples of one of the suitable aspects of those other resins include a resin having a polymerizable group such as an unsaturated double bond (for example, an ethylenically unsaturated double bond), an epoxy group, or an oxetanyl group. In a case where the polymerizable group reacts in the process of forming a magnetic particle-containing film, a magnetic particle-containing film having excellent mechanical strength is obtained.

Examples of those other resins include a polymer having an epoxy group on a side chain and a polymerizable monomer or oligomer having two or more epoxy groups in the molecule. Specific examples thereof include a bisphenol A-type epoxy resin, a bisphenol F-type epoxy resin, a phenol novolac-type epoxy resin, a cresol novolac-type epoxy resin, an aliphatic epoxy resin, and the like.

As these other resins, commercially available products may also be used. Furthermore, these resins may be obtained by introducing an epoxy group into a side chain of a polymer.

As for the commercially available products, for example, the description in paragraph "0191" of JP2012-155288A and the like can be referred to, and what are described in the paragraph are incorporated into the present specification.

Examples of the commercially available product also include ADEKA RESIN EP-4000S, ADEKA RESIN EP-4003S, ADEKA RESIN EP-4010S, and ADEKA RESIN EP-4011S (all are manufactured by ADEKA CORPORATION), NC-2000, NC-3000, NC-7300, XD-1000, EPPN-501, and EPPN-502 (all are manufactured by ADEKA CORPORATION), JER103 1S, and the like.

Examples of commercially available products of the phenol novolac-type epoxy resin include JER-157S65, JER-152, JER-154, and JER-157S70 (all are manufactured by Mitsubishi Chemical Holdings Corporation.) and the like.

Specifically, as the polymer having an oxetanyl group on a side chain and the aforementioned polymerizable monomer or oligomer having two or more oxetanyl groups in the molecule, for example, ARON OXETANE OXT-121, OXT-221, OX-SQ, and PNOX (all are manufactured by TOAGOSEI CO., LTD.) can be used.

In a case where an epoxy group is introduced into a side chain of a polymer such that those other resins having an epoxy group are synthesized, the introduction reaction is performed by causing the reaction in an organic solvent at a reaction temperature of 50°C to 150°C for a predetermined time by using, for example, a tertiary amine such as triethylamine or benzylmethylamine, a quaternary ammonium salt such as dodecyltrimethylammonium chloride, tetramethylammonium chloride, or tetraethylammonium chloride, pyridine, triphenylphosphine or the like as a catalyst. The amount of the alicyclic epoxy unsaturated compound to be introduced can be controlled such that the acid value of the obtained polymer falls into a range of 5 to 200 KOH·mg/g. The weight-average molecular weight can be in a range of 500 to 5,000,000, and preferably in a range of 1,000 to 500,000.

Instead of the alicyclic epoxy unsaturated compound, it is also possible to use a compound having a glycidyl group as an epoxy group, such as glycidyl (meth)acrylate or allyl glycidyl ether. As for such a compound, for example, the description in paragraph "0045" of JP2009-265518A and the like can be referred to, and what are described in the paragraph are incorporated into the present specification.

Examples of one of the suitable aspects of those other resins include other resins having an acid group, a basic group, or an amide group. In view of further improving the effects of the present invention, the aforementioned other resins having an acid group, a basic group, or an amide group are suitable because these resins are likely to function as a dispersant for dispersing the magnetic particles.

Examples of the acid group include a carboxy group, a phosphoric acid group, a sulfo group, a phenolic hydroxyl group, and the like. In view of further improving the effects of the present invention, a carboxy group is preferable.

Examples of the basic group include an amino group (ammonia, a group obtained by removing one hydrogen atom from a primary amine or a secondary amine) and an imino group.

In view of further improving the effects of the present invention, it is preferable that those other resins have a carboxy group or an amide group among the above.

In a case where those other resins have an acid group, in view of further improving the effects of the present invention, the acid value of those other resins is preferably 10 to 500 mgKOH/g, and particularly preferably 30 to 400 mgKOH/g.

In view of further improving the dispersibility of those other resins in the composition such that the effects of the present invention are further improved, as those other resins to be used, other resins having a solubility of 10 g/L or more in a solvent are preferable, and other resins having a solubility of 20 g/L or more in a solvent are more preferable.

The upper limit of the solubility of those other resins in a solvent is preferably 2,000 g/L or less, and particularly preferably 1,000 g/L or less.

The solubility of a resin in a solvent means the amount (g) of the resin dissolved in 1 L of a solvent at 25°C.

In view of further improving the effects of the present invention, the content of those other resins with respect to the total mass of the composition is preferably 0.1% to 30% by mass, more preferably 1% to 20% by mass, even more preferably 2% to 15% by mass, and particularly preferably 2.5% to 10% by mass.

The content of those other resins with respect to the total solid content of the composition is preferably 0.1% to 30% by mass, more preferably 1% to 20% by mass, even more preferably 2% to 15% by mass, and particularly preferably 2.5% to 10% by mass.

### <Resin having repeating unit having graft chain (resin A)>

Examples of those other resins include a resin having a repeating unit having a graft chain (hereinafter, this resin will be also called "resin A"). The resin A can assist the effect of the rheology control agent and improve the effect of improving temporal stability of the composition.

In a case where the composition contains the resin A, in view of further improving the effects of the present invention, the content of the resin A with respect to the total mass of the composition is preferably 0.1% to 30% by mass, more preferably 0.5% to 20% by mass, and even more preferably 1% to 10% by mass.

The content of the resin A with respect to the total solid content of the composition is preferably 0.1% to 30% by mass, more preferably 0.5% to 20% by mass, and even more preferably 1% to 10% by mass.

In a case where the resin A is used, the mass ratio of the content of the rheology control agent to the content of the resin A (rheology control agent/resin A) is preferably 10/90 to 90/10, more preferably 30/70 to 80/20, and even more preferably 50/50 to 70/30.

### (Repeating unit having graft chain)

The longer the graft chain in the repeating unit having a graft chain, the higher the effect of steric repulsion, which improves the dispersibility of the specific magnetic particles. In contrast, in a case where the graft chain is too long, the adsorptive force with respect to the specific magnetic particles is reduced, which tends to deteriorate the dispersibility of the specific magnetic particles. Therefore, the number of atoms constituting the graft chain excluding a hydrogen atom is preferably 40 to 10,000, more preferably 50 to 2,000, and even more preferably 60 to 500.

The graft chain mentioned herein refers to a portion from the root of the main chain (atom bonded to the main chain in a group branching off from the main chain) to the terminal of the group branching off from the main chain.

It is preferable that the graft chain contain a polymer structure. Examples of such a polymer structure include a poly(meth)acrylate structure (for example, a poly(meth)acrylic structure), a polyester structure, a polyurethane structure, a polyurea structure, a polyamide structure, a polyether structure, and the like.

In order to improve the interactivity between the graft chain and a solvent such that the dispersibility of the specific magnetic particles is improved, the graft chain is preferably a graft chain containing at least one structure selected from the group consisting of a polyester structure, a polyether structure, and a poly(meth)acrylate structure, and more preferably a graft chain containing at least either a polyester structure or a polyether structure.

The resin A may be a resin obtained using a macromonomer having a graft chain (a monomer that has a polymer structure and is bonded to a main chain to constitute a graft chain).

The macromonomer having a graft chain (monomer that has a polymer structure and is bonded to a main chain to constitute a graft chain) is not particularly limited. As this macromonomer, a macromonomer containing a reactive double bond-forming group can be suitably used.

As commercially available macromonomers that correspond to the aforementioned repeating unit having a graft chain and suitably used for the synthesis of the resin A, AA-6, AA-10, AB-6, AS-6, AN-6, AW-6, AA-714, AY-707, AY-714, AK-5, AK-30, and AK-32 (all are trade names, manufactured by TOAGOSEI CO., LTD.), and BLEMMER PP-100, BLEMMER PP-500, BLEMMER PP-800, BLEMMER PP-1000, BLEMMER 55-PET-800, BLEMMER PME-4000, BLEMMER PSE-400, BLEMMER PSE-1300, and BLEMMER 43PAPE-600B (all are trade names, manufactured by NOF CORPORATION.) are used. Among these, AA-6, AA-10, AB-6, AS-6, AN-6, or BLEMMER PME-4000 is preferable.

The resin A preferably contains at least one structure selected from the group consisting of polymethyl acrylate, polymethyl methacrylate, and cyclic or chain-like polyester, more preferably contains at least one structure selected from the group consisting of polymethyl acrylate, polymethyl methacrylate, and chain-like polyester, and even more preferably contains at least one structure selected from the group consisting of a polymethyl acrylate structure, a polymethyl methacrylate structure, a polycaprolactone structure, and a polyvalerolactone structure. The resin A may contain only one structure described above or a plurality of structures described above.

The polycaprolactone structure mentioned herein refers to a structure containing, as a repeating unit, a structure formed by ring opening of ε-caprolactone. The polyvalerolactone structure refers to a structure containing, as a repeating unit, a structure formed by ring opening of δ-valerolactone.

In a case where the resin A contains repeating units represented by Formula (1) and Formula (2), which will be described later, where each of j and k is 5, the aforementioned polycaprolactone structure can be introduced into the resin A.

In a case where the resin A contains repeating units represented by Formula (1) and Formula (2), which will be described later, where each of j and k is 4, the aforementioned polyvalerolactone structure can be introduced into the resin A.

In a case where the resin A contains a repeating unit represented by Formula (4), which will be described later, where X⁵ is a hydrogen atom and R⁴ is a methyl group, the aforementioned polymethyl acrylate structure can be introduced into the resin A.

In a case where the resin A contains a repeating unit represented by Formula (4), which will be described later, where X⁵ and R⁴ both represent a methyl group, the aforementioned polymethyl methacrylate structure can be introduced into the resin A.

As the repeating unit having a graft chain that the resin A is to contain, a repeating unit represented by any of the following Formula (1) to Formula (4) is preferable, and a repeating unit represented by any of the following Formula (1A), the following Formula (2A), the following Formula (3A), the following Formula (3B), and the following Formula (4) is more preferable.

In Formulas (1) to (4), W¹, W², W³, and W⁴ each independently represent an oxygen atom or NH. W¹, W², W³, and W⁴ are preferably oxygen atoms.

In Formulas (1) to (4), X¹, X², X³, X⁴, and X⁵ each independently represent a hydrogen atom or a monovalent organic group. In view of restrictions on synthesis, X¹, X², X³, X⁴, and X⁵ preferably each independently represent a hydrogen atom or an alkyl group with a carbon number (the number of carbon atoms) of 1 to 12, more preferably each independently represent a hydrogen atom or a methyl group, and even more preferably each independently represent a methyl group.

In Formulas (1) to (4), Y¹, Y², Y³, and Y⁴ each independently represent a divalent linking group. The structure of the linking group is not particularly restricted. Specific examples of the divalent linking group represented by Y¹, Y², Y³, and Y⁴ include the following linking groups (Y-1) to (Y-21) and the like. In the following structures, A means a bonding site to the left terminal group in Formulas (1) to (4), and B means a bonding site to the right terminal group in Formulas (1) to (4). Among the following structures, in view of ease of synthesis, (Y-2) or (Y-13) is more preferable.

In Formulas (1) to (4), Z¹, Z², Z³, and Z⁴ each independently represent a hydrogen atom or a monovalent substituent. The structure of the substituent is not particularly limited. Specific examples of the substituent include an alkyl group, a hydroxyl group, an alkoxy group, an aryloxy group, a heteroaryloxy group, an alkylthioether group, an arylthioether group, a heteroarylthioether group, an amino group, and the like. Among these, as the group represented by Z¹, Z², Z³, and Z⁴, particularly, in view of improving dispersibility, a group that brings about a steric repulsion effect is preferable. Z¹, Z², Z³, and Z⁴ more preferably each independently represent an alkyl or alkoxy group with a carbon number of 5 to 24. Especially, Z¹, Z², Z³, and Z⁴ even more preferably each independently represent a branched alkyl group with a carbon number of 5 to 24, a cyclic alkyl group with a carbon number of 5 to 24, or an alkoxy group with a carbon number of 5 to 24. Note that the alkyl group contained in the alkoxy group may be linear, branched, or cyclic.

The substituent represented by Z¹, Z², Z³, and Z⁴ is also preferably a group containing a curable group such as a (meth)acryloyl group, an epoxy group, and/or an oxetanyl group. Examples of the group containing a curable group include "-O-alkylene group-(-O-alkylene group-)_{AL}-(meth)acryloyloxy group". AL represents an integer of 0 to 5. AL is preferably 1. The aforementioned alkylene group preferably each independently has a carbon number of 1 to 10. In a case where the alkylene group has a substituent, the substituent is preferably a hydroxyl group.

The substituent may be a group containing an onium structure.

The group containing an onium structure is a group having an anionic moiety and a cationic moiety. Examples of the anionic moiety include a partial structure containing an oxygen anion (-O⁻). Particularly, the oxygen anion (-O⁻) is preferably directly bonded to the terminal of the repeating structure having n, m, p, or q in the repeating unit represented by any of Formulas (1) to (4), and more preferably directly bonded to the terminal of the repeating structure having n in the repeating unit represented by Formula (1) (that is, the right terminal in -(-O-CⱼH₂ⱼ-CO-)ₙ-).

Examples of the cation in the cationic moiety of the group containing an onium structure include an ammonium cation. In a case where the cationic moiety is an ammonium cation, the cationic moiety is a partial structure containing a cationic nitrogen atom (>N⁺<). The cationic nitrogen atom (>N⁺<) is preferably bonded to 4 substituents (preferably organic groups), and 1 to 4 out of the substituents are preferably an alkyl group with a carbon number of 1 to 15. One or more out of the 4 substituents (preferably one of the 4 substituents) are also preferably a group containing a curable group such as a (meth)acryloyl group, an epoxy group, and/or an oxetanyl group. Examples of the group containing a curable group that can be the substituent include "-O-alkylene group-(-O-alkylene group-)_{AL}-(meth)acryloyloxy group" described above.

In Formulas (1) to (4), n, m, p, and q each independently represent an integer of 1 to 500.

In Formulas (1) and (2), j and k each independently represent an integer of 2 to 8. Each of j and k in Formulas (1) and (2) is preferably an integer of 4 to 6, and more preferably 5.

In Formulas (1) and (2), each of n and m is, for example, an integer of 2 or more, preferably an integer of 6 or more, more preferably an integer of 10 or more, and even more preferably an integer of 20 or more. In a case where the resin A contains a polycaprolactone structure and a polyvalerolactone structure, the sum of the repetition number of the polycaprolactone structure and the repetition number of polyvalerolactone is preferably an integer of 10 or more, and more preferably an integer of 20 or more.

In Formula (3), R³ represents a branched or linear alkylene group which is preferably an alkylene group with a carbon number of 1 to 10, and more preferably an alkylene group with a carbon number of 2 or 3. In a case where p is 2 to 500, a plurality of R³'s may be the same or different from each other.

In Formula (4), R⁴ represents a hydrogen atom or a monovalent organic group, and the structure of the monovalent substituent is not particularly limited. R⁴ is preferably a hydrogen atom, an alkyl group, an aryl group, or a heteroaryl group, and more preferably a hydrogen atom or an alkyl group. In a case where R⁴ is an alkyl group, the alkyl group is preferably a linear alkyl group with a carbon number of 1 to 20, a branched alkyl group with a carbon number of 3 to 20, or a cyclic alkyl group with a carbon number of 5 to 20, more preferably a linear alkyl group with a carbon number of 1 to 20, and even more preferably a linear alkyl group with a carbon number of 1 to 6. In a case where q in Formula (4) is 2 to 500, a plurality of X⁵'s and R⁴'s in the graft chain may be the same or different from each other.

The resin A may contain two or more repeating units having different structures and having a graft chain. That is, the molecule of the resin A may contain repeating units represented by Formulas (1) to (4) having different structures. Furthermore, in a case where n, m, p, and q in Formulas (1) to (4) each represent an integer of 2 or more, the side chains in Formulas (1) and (2) may contain structures where j and k represent different integers, and a plurality of R³'s, R⁴'s, and X⁵'s in the molecules of Formulas (3) and (4) may be the same or different from each other.

The repeating unit represented by Formula (1) is more preferably a repeating unit represented by the following Formula (1A).

The repeating unit represented by Formula (2) is more preferably a repeating unit represented by the following Formula (2A).

X¹, Y¹, Z¹, and n in Formula (1A) have the same definitions as X¹, Y¹, Z¹, and n in Formula (1), and preferable ranges thereof are the same as well. X², Y², Z², and m in Formula (2A) have the same definitions as X², Y², Z², and m in Formula (2), and preferable ranges thereof are the same as well.

The repeating unit represented by Formula (3) is more preferably a repeating unit represented by the following Formula (3A) or the following Formula (3B).

X³, Y³, Z³, and p in Formula (3A) or (3B) have the same definitions as X³, Y³, Z³, and p in Formula (3), and preferable ranges thereof are the same as well.

It is more preferable that the resin A contain the repeating unit represented by Formula (1A) as the repeating unit having a graft chain.

It is also preferable that the resin A contain a repeating unit containing a polyalkylene imine structure and a polyester structure. It is preferable that the repeating unit containing a polyalkylene imine structure and a polyester structure contain the polyalkylene imine structure on the main chain and contain the polyester structure as a graft chain.

The polyalkylene imine structure is a polymerization structure having two or more identical or different alkylene imine chains. Specific examples of the alkylene imine chain include alkylene imine chains represented by the following Formula (4A) and the following Formula (4B).

In Formula (4A), R^{x1} and R^{x2} each independently represent a hydrogen atom or an alkyl group. a¹ represents an integer of 2 or more. ^{∗1} represents a bonding position to a polyester chain, an adjacent alkylene imine chain, a hydrogen atom, or a substituent.

In Formula (4B), R^{x3} and R^{x4} each independently represent a hydrogen atom or an alkyl group. a² represents an integer of 2 or more. The alkylene imine chain represented by Formula (4B) is bonded to a polyester chain having an anionic group by the formation of a salt crosslinking group of N⁺ shown in Formula (4B) and an anionic group contained in the polyester chain.
* in Formula (4A) and Formula (4B) and ^{∗2} in Formula (4B) each independently represent a position to be bonded to an adjacent alkylene imine chain, a hydrogen atom, or a substituent.
* in Formula (4A) and Formula (4B) particularly preferably represent a position to be bonded to an adjacent alkylene imine chain.

R^{X1} and R^{X2} in Formula (4A) and R^{X3} and R^{X4} in Formula (4B) each independently represent a hydrogen atom or an alkyl group.

The carbon number of the alkyl group is preferably 1 to 6, and more preferably 1 to 3.

It is preferable that R^{X1} and R^{X2} in Formula (4A) both represent a hydrogen atom.

It is preferable that R^{X3} and R^{X4} in Formula (4B) both represent a hydrogen atom.

a¹ in Formula (4A) and a² in Formula (4B) are not particularly limited as long as a¹ and a² each represent an integer of 2 or more. The upper limit of a¹ and a² is preferably 10 or less, more preferably 6 or less, even more preferably 4 or less, still more preferably 2 or 3, and particularly preferably 2.
* in Formula (4A) and Formula (4B) represents a bonding position to an adjacent alkylene imine chain, a hydrogen atom, or a substituent.

Examples of the aforementioned substituent include a substituent such as an alkyl group (for example, an alkyl group with a carbon number of 1 to 6). Furthermore, a polyester chain may be bonded thereto as a substituent.

The alkylene imine chain represented by Formula (4A) is preferably linked to the polyester chain at the position represented by ^{∗1} described above. Specifically, it is preferable that the carbonyl carbon in the polyester chain be bonded at the position represented by ^{∗1} described above.

Examples of the polyester chain include a polyester chain represented by the following formula (5A).

In a case where the alkylene imine chain is an alkylene imine chain represented by Formula (4B), it is preferable that the polyester chain contain an anion (preferably an oxygen anion O⁻), and that the anion and N⁺ in Formula (4B) form a salt crosslinking group.

Examples of such a polyester chain include a polyester chain represented by the following Formula (5B).

L^{X1} in Formula (5A) and L^{X2} in Formula (5B) each independently represent a divalent linking group. Preferred examples of the divalent linking group include an alkylene group with a carbon number of 3 to 30.

b¹¹ in Formula (5A) and b²¹ in Formula (5B) each independently represent an integer of 2 or more. Each of b¹¹ and b²¹ is preferably an integer of 6 or more, and the upper limit thereof is, for example, 200 or less.

b¹² in Formula (5A) and b²² in Formula (5B) each independently represent 0 or 1.

X^{A} in Formula (5A) and X^{B} in Formula (5B) each independently represent a hydrogen atom or a substituent. Examples of the substituent include an alkyl group, an alkoxy group, a polyalkyleneoxyalkyl group, an aryl group, and the like.

The carbon number of the aforementioned alkyl group (the alkyl group may be any of linear, branch, and cyclic alkyl groups) and the carbon number of an alkyl group (the alkyl group may be any of linear, branch, and cyclic alkyl groups) contained in the aforementioned alkoxy group are, for example, 1 to 30, and preferably 1 to 10. The aforementioned alkyl group may further have a substituent. Examples of the substituent include a hydroxyl group and a halogen atom (the halogen atom includes a fluorine atom, a chlorine atom, a bromine atom, an iodine atom, and the like).

The polyalkyleneoxyalkyl group is a substituent represented by R^{X6}(OR^{X7})ₚ(O)_{q}-. R^{X6} represents an alkyl group, R^{X7} represents an alkylene group, p represents an integer of 2 or more, and q represents 0 or 1.

The alkyl group represented by R^{X6} has the same definition as the alkyl group represented by X^{A}. Examples of the alkylene group represented by R^{X7} include a group obtained by removing one hydrogen atom from the alkyl group represented by X^{A}.
p is an integer of 2 or more, and the upper limit thereof is, for example, 10 or less, and preferably 5 or less.

Examples of the aryl group include an aryl group (which may be monocyclic or polycyclic) with a carbon number of 6 to 24.

The aforementioned aryl group may further have a substituent. Examples of the substituent include an alkyl group, a halogen atom, a cyano group, and the like.

The aforementioned polyester chain is preferably a structure established by ring opening of lactones such as ε-caprolactone, δ-caprolactone, β-propiolactone, γ-butyrolactone, δ-valerolactone, γ-valerolactone, enanthonolactone, β-butyrolactone, γ-hexanolactone, γ-octanolactone, δ-hexanolactone, δ-octanolactone, δ-dodecanolactone, α-methyl-γ-butyrolactone, and lactide (which may be L-lactide or D-lactide), and more preferably a structure established by ring opening of ε-caprolactone or δ-valerolactone.

The aforementioned repeating unit containing a polyalkylene imine structure and a polyester structure can be synthesized according to the synthesis method described in JP5923557B.

In the resin A, the content of the repeating unit having a graft chain expressed in terms of mass with respect to the total mass of the resin A is, for example, 2% to 100% by mass, preferably 2% to 95% by mass, more preferably 2% to 90% by mass, and even more preferably 5% to 30% by mass. In a case where the content of the repeating unit having a graft chain is in this range, the effects of the present invention are further improved.

### (Hydrophobic repeating unit)

The resin A may contain a hydrophobic repeating unit that is different from the repeating unit having a graft chain (that is, does not correspond to the repeating unit having a graft chain). In the present specification, the hydrophobic repeating unit refers to a repeating unit having no acid group (for example, a carboxylic acid group, a sulfonic acid group, a phosphoric acid group, a phenolic hydroxyl group, and the like).

The hydrophobic repeating unit is preferably a repeating unit derived from (corresponding to) a compound (monomer) having a ClogP value of 1.2 or more, and is more preferably a repeating unit derived from a compound having a ClogP value of 1.2 to 8. In a case where this hydrophobic repeating unit is used, the effects of the present invention can be more reliably expressed.

The ClogP value is a value calculated by a program "CLOGP" available from Daylight Chemical Information System, Inc. This program provides a value of "calculated logP" calculated by the fragment approach (see the following documents) of Hansch and Leo. The fragment approach is based on the chemical structure of a compound. In this method, the chemical structure is divided into partial structures (fragments), and degrees of contribution to logP that are assigned to the fragments are summed up, thereby estimating the logP value of the compound. Details of the method are described in the following documents. In the present specification, a ClogP value calculated by a program CLOGP v 4.82 is used.

A. J. Leo, Comprehensive Medicinal Chemistry, Vol. 4, C. Hansch, P. G. Sammnens, J. B. Taylor and C. A. Ramsden, Eds., p. 295, Pergamon press, 1990, C. Hansch & A. J. Leo. Substituent Constants For Correlation Analysis in Chemistry and Biology. John Wiley & Sons. A. J. Leo. Calculating logPoct from structure. Chem. Rev., 93, 1281-1306, 1993.

logP means a common logarithm of a partition coefficient P. logP is a value of physical properties that shows how a certain organic compound is partitioned in an equilibrium of two-phase system consisting of oil (generally, 1-octanol) and water by using a quantitative numerical value. logP is represented by the following equation. $logP = log \left(Coil/Cwater\right)$

In the formula, Coil represents a molar concentration of a compound in an oil phase, and Cwater represents a molar concentration of the compound in a water phase.

The greater the positive logP value based on 0, the higher the oil solubility. The greater the absolute value of negative logP, the higher the water solubility. The value of logP is negatively correlated with the water solubility of an organic compound, and widely used as a parameter for estimating the hydrophilicity and hydrophobicity of an organic compound.

It is preferable that the resin A contain, as the hydrophobic repeating unit, one or more repeating units selected from repeating units derived from the monomers represented by the following Formulas (i) to (iii).

In the above Formulas (i) to (iii), R¹, R², and R³ each independently represent a hydrogen atom, a halogen atom (for example, a fluorine atom, a chlorine atom, a bromine atom, or the like), or an alkyl group with a carbon number of 1 to 6 (for example, a methyl group, an ethyl group, a propyl group, or the like).

Each of R¹, R², and R³ is preferably a hydrogen atom or an alkyl group with a carbon number of 1 to 3, and more preferably a hydrogen atom or a methyl group. Each of R² and R³ is even more preferably a hydrogen atom.

X represents an oxygen atom (-O-) or an imino group (-NH-), and is preferably an oxygen atom.

L represents a single bond or a divalent linking group. Examples of the divalent linking group include a divalent aliphatic group (for example, an alkylene group, a substituted alkylene group, an alkenylene group, a substituted alkenylene group, an alkynylene group, or a substituted alkynylene group), a divalent aromatic group (for example, an arylene group or a substituted arylene group), a divalent heterocyclic group, an oxygen atom (-O-), a sulfur atom (-S-), an imino group (-NH-), a substituted imino group (-NR³¹-, where R³¹ is an aliphatic group, an aromatic group, or a heterocyclic group), a carbonyl group (-CO-), a combination of these, and the like.

The divalent aliphatic group may have a cyclic structure or a branched structure. The carbon number of the aliphatic group is preferably 1 to 20, more preferably 1 to 15, and even more preferably 1 to 10. The aliphatic group may be an unsaturated aliphatic group or a saturated aliphatic group, and is preferably a saturated aliphatic group. Furthermore, the aliphatic group may have a substituent. Examples of the substituent include a halogen atom, an aromatic group, a heterocyclic group, and the like.

The carbon number of the divalent aromatic group is preferably 6 to 20, more preferably 6 to 15, and even more preferably 6 to 10. Furthermore, the aromatic group may have a substituent. Examples of the substituent include a halogen atom, an aliphatic group, an aromatic group, a heterocyclic group, and the like.

It is preferable that the divalent heterocyclic group contain a 5-membered ring or a 6-membered ring as the heterocycle. Another heterocycle, aliphatic ring, or aromatic ring may be condensed with the heterocycle. Furthermore, the heterocyclic group may have a substituent. Examples of the substituent include a halogen atom, a hydroxyl group, an oxo group (=O), a thioxo group (=S), an imino group (=NH), a substituted imino group (=N-R³², where R³² is an aliphatic group, an aromatic group, or a heterocyclic group), an aliphatic group, an aromatic group, and a heterocyclic group.

L is preferably a single bond or a divalent linking group containing an alkylene group or an oxyalkylene structure. The oxyalkylene structure is more preferably an oxyethylene structure or an oxypropylene structure. Furthermore, L may contain a polyoxyalkylene structure containing two or more repeating oxyalkylene structures. As the polyoxyalkylene structure, a polyoxyethylene structure or a polyoxypropylene structure is preferable. The polyoxyethylene structure is represented by -(OCH₂CH2)n-. n is preferably an integer of 2 or more, and more preferably an integer of 2 to 10.

Examples of Z include an aliphatic group (for example, an alkyl group, a substituted alkyl group, an unsaturated alkyl group, or a substituted unsaturated alkyl group), an aromatic group (for example, an aryl group, a substituted aryl group, an arylene group, or a substituted arylene group), a heterocyclic group, and a combination of these. These groups may contain an oxygen atom (-O-), a sulfur atom (-S-), an imino group (-NH-), a substituted imino group (-NR³¹-, where R³¹ is an aliphatic group, an aromatic group, or a heterocyclic group), or a carbonyl group (-CO-).

The aliphatic group may have a cyclic structure or a branched structure. The carbon number of the aliphatic group is preferably 1 to 20, more preferably 1 to 15, and even more preferably 1 to 10. The aliphatic group further contains a ring assembly hydrocarbon group and a crosslinked cyclic hydrocarbon group. Examples of the ring assembly hydrocarbon group include a bicyclohexyl group, a perhydronaphthalenyl group, a biphenyl group, a 4-cyclohexylphenyl group, and the like. Examples of a crosslinked cyclic hydrocarbon ring include a bicyclic hydrocarbon ring such as a pinane, bornane, norpinane, norbornane, or bicyclooctane ring (such as a bicyclo[2.2.2]octane ring or a bicyclo[3.2.1]octane ring), a tricyclic hydrocarbon ring such as a homobredane, adamantane, tricyclo[5.2.1.0^{2,6}]decane, or tricyclo[4.3.1.1^{2,5}]undecane ring, a tetracyclic hydrocarbon ring such as a tetracyclo[4.4.0.1^{2,5}.1^{7,10}]dodecane or perhydro-1,4-methano-5,8-methanonaphthalene ring, and the like. In addition, the crosslinked cyclic hydrocarbon ring also includes fused hydrocarbon rings, for example, fused rings consisting of a plurality of condensed 5- to 8-membered cycloalkane rings such as perhydronaphthalene (decalin), perhydroanthracene, perhydrophenanthrene, perhydroacenaphtene, perhydrofluorene, perhydroindene, and perhydrophenanthrene rings.

As the aliphatic group, a saturated aliphatic group is preferred over an unsaturated aliphatic group. Furthermore, the aliphatic group may have a substituent. Examples of the substituent thereof include a halogen atom, an aromatic group, and a heterocyclic group. Here, the aliphatic group does not have an acid group as a substituent.

The carbon number of the aromatic group is preferably 6 to 20, more preferably 6 to 15, and even more preferably 6 to 10. Furthermore, the aromatic group may have a substituent. Examples of the substituent include a halogen atom, an aliphatic group, an aromatic group, and a heterocyclic group. Here, the aromatic group does not have an acid group as a substituent.

It is preferable that the heterocyclic group contain a 5-membered ring or a 6-membered ring as the heterocycle. Another heterocycle, aliphatic ring, or aromatic ring may be condensed with the heterocycle. Furthermore, the heterocyclic group may have a substituent. Examples of the substituent include a halogen atom, a hydroxyl group, an oxo group (=O), a thioxo group (=S), an imino group (=NH), a substituted imino group (=N-R³², where R³² is an aliphatic group, an aromatic group, or a heterocyclic group), an aliphatic group, an aromatic group, and a heterocyclic group. Here, the heterocyclic group does not have an acid group as a substituent.

In the above Formula (iii), R⁴, R⁵, and R⁶ each independently represent a hydrogen atom, a halogen atom (for example, a fluorine atom, a chlorine atom, a bromine atom, or the like), an alkyl group with a carbon number of 1 to 6 (for example, a methyl group, an ethyl group, a propyl group, or the like), Z, or L-Z. Here, L and Z have the same definition as the aforementioned groups represented by L and Z. Each of R⁴, R⁵, and R⁶ is preferably a hydrogen atom or an alkyl group with a carbon number of 1 to 3, and more preferably a hydrogen atom.

As the monomer represented by the above Formula (i), a compound is preferably in which each of R¹, R², and R³ is a hydrogen atom or a methyl group, L is a single bond or a divalent linking group containing an alkylene group or an oxyalkylene structure, X is an oxygen atom or an imino group, and Z is an aliphatic group, a heterocyclic group, or an aromatic group.

As the monomer represented by the above Formula (ii), a compound is preferable in which R¹ is a hydrogen atom or a methyl group, L is an alkylene group, and Z is an aliphatic group, a heterocyclic group, or an aromatic group. Furthermore, as the monomer represented by the above Formula (iii), a compound is preferable in which each of R⁴, R⁵, and R⁶ is a hydrogen atom or a methyl group, and Z is an aliphatic group, a heterocyclic group, or an aromatic group.

Examples of typical compounds represented by Formulas (i) to (iii) include a radically polymerizable compound selected from acrylic acid esters, methacrylic acid esters, styrenes, and the like.

As examples of the typical compounds represented by Formulas (i) to (iii), the compounds described in paragraphs "0089" to "0093" of JP2013-249417A can be referred to, and what are described in the paragraphs are incorporated into the present specification.

In the resin A, the content of the hydrophobic repeating unit, expressed in terms of mass, with respect to the total mass of the resin A is preferably 10% to 90% by mass, and more preferably 20% to 80% by mass.

### (Functional group capable of interacting with specific magnetic particles)

The resin A may have a functional group capable of interacting with the specific magnetic particles.

It is preferable that the resin A further contain a repeating unit containing a functional group that is capable of interacting with the specific magnetic particles.

Examples of the functional group capable of interacting with the specific magnetic particles include an acid group, a basic group, a coordinating group, a reactive functional group, and the like.

In a case where the resin A contains an acid group, a basic group, a coordinating group, or a reactive functional group, it is preferable that the resin A contain a repeating unit containing an acid group, a repeating unit containing a basic group, a repeating unit containing a coordinating group, or a repeating unit having a reactive functional group.

The repeating unit containing an acid group may be a repeating unit that is the same as or different from the aforementioned repeating unit having a graft chain. However, the repeating unit containing an acid group is a repeating unit different from the aforementioned hydrophobic repeating unit (that is, does not correspond to the aforementioned hydrophobic repeating unit).

Examples of the acid group which is a functional group capable of interacting with the specific magnetic particles include a carboxylic acid group, a sulfonic acid group, a phosphoric acid group, a phenolic hydroxyl group, and the like. The acid group is preferably at least one group among a carboxylic acid group, a sulfonic acid group, and a phosphoric acid group, and more preferably a carboxylic acid group. The carboxylic acid group has excellent adsorptive force with respect to the specific magnetic particles and has high dispersibility.

That is, it is preferable that the resin A further contain a repeating unit containing at least one group among a carboxylic acid group, a sulfonic acid group, and a phosphoric acid group.

The resin A may have one repeating unit containing an acid group or two or more such repeating units.

In a case where the resin A contains the repeating unit containing an acid group, the content of the repeating unit expressed in terms of mass with respect to the total mass of the resin A is preferably 5% to 80% by mass, and more preferably 10% to 60% by mass.

Examples of the basic group which is a functional group capable of interacting with the specific magnetic particles include a primary amino group, a secondary amino group, a tertiary amino group, a heterocycle containing a N atom, an amide group, and the like. As the basic group, in view of excellent adsorptive force with respect to the specific magnetic particles and high dispersibility, a tertiary amino group is preferable. The resin A may contain one basic group described above or two or more basic groups described above.

In a case where the resin A contains the repeating unit containing a basic group, the content of the repeating unit expressed in terms of mass with respect to the total mass of the resin A is preferably 0.01% to 50% by mass, and more preferably 0.01% to 30% by mass.

Examples of the coordinating group and the reactive functional group which are functional groups capable of interacting with the specific magnetic particles include an acetylacetoxy group, a trialkoxysilyl group, an isocyanate group, an acid anhydride, an acid chloride, and the like. As these functional groups, in view of excellent adsorptive force with respect to the specific magnetic particles and high dispersibility of the specific magnetic particles, an acetylacetoxy group is preferable. The resin A may have one of these groups or two or more of these groups.

In a case where the resin A contains the repeating unit containing a coordinating group or the repeating unit containing a reactive functional group, the content of the repeating unit expressed in terms of mass with respect to the total mass of the resin A is preferably 10% to 80% by mass, and more preferably 20% to 60% by mass.

In a case where the resin A contains, in addition to a graft chain, a functional group capable of interacting with the specific magnetic particles, the resin A may contain a functional group capable of interacting with various specific magnetic particles described above, and the way the functional group is introduced into the resin A is not particularly limited. For example, it is preferable that the resin to be incorporated into the composition contain one or more repeating units selected from repeating units derived from the monomers represented by the following Formulas (iv) to (vi).

In Formulas (iv) to (vi), R¹¹, R¹², and R¹³ each independently represent a hydrogen atom, a halogen atom (for example, a fluorine atom, a chlorine atom, a bromine atom, or the like), or an alkyl group with a carbon number of 1 to 6 (for example, a methyl group, an ethyl group, a propyl group, or the like).

In Formulas (iv) to (vi), each of R¹¹, R¹², and R¹³ is preferably a hydrogen atom or an alkyl group with a carbon number of 1 to 3, and more preferably a hydrogen atom or a methyl group. Each of R¹² and R¹³ in Formula (iv) is even more preferably a hydrogen atom.

X₁ in Formula (iv) represents an oxygen atom (-O-) or an imino group (-NH-), and is preferably an oxygen atom.

Y in Formula (v) represents a methine group or a nitrogen atom.

L₁ in Formulas (iv) to (v) represents a single bond or a divalent linking group. The divalent linking group has the same definition as the divalent linking group represented by L in Formula (i) described above.

L₁ is preferably a single bond or a divalent linking group containing an alkylene group or an oxyalkylene structure. The oxyalkylene structure is more preferably an oxyethylene structure or an oxypropylene structure. Furthermore, L₁ may contain a polyoxyalkylene structure including two or more repeating oxyalkylene structures. As the polyoxyalkylene structure, a polyoxyethylene structure or a polyoxypropylene structure is preferable. The polyoxyethylene structure is represented by -(OCH₂CH₂)n-. n is preferably an integer of 2 or more, and more preferably an integer of 2 to 10.

In Formulas (iv) to (vi), Z₁ represents a functional group that is capable of interacting with the specific magnetic particles as well in addition to the graft chain. Z₁ is preferably a carboxylic acid group or a tertiary amino group, and more preferably a carboxylic acid group.

In Formula (vi), R¹⁴, R¹⁵, and R¹⁶ each independently represent a hydrogen atom, a halogen atom (for example, a fluorine atom, a chlorine atom, a bromine atom, or the like), an alkyl group with a carbon number of 1 to 6 (for example, a methyl group, an ethyl group, a propyl group, or the like), -Z₁, or L₁-Z₁. Here, L₁ and Z₁ have the same definitions as L₁ and Z₁ described above, and preferred examples thereof are also the same. Each of R¹⁴, R¹⁵, and R¹⁶ is preferably a hydrogen atom or an alkyl group with a carbon number of 1 to 3, and more preferably a hydrogen atom.

As the monomer represented by Formula (iv), a compound is preferable in which R¹¹, R¹², and R¹³ each independently represent a hydrogen atom or a methyl group, L¹ is a divalent linking group containing an alkylene group or an oxyalkylene structure, X₁ is an oxygen atom or an imino group, and Z₁ is a carboxylic acid group.

As the monomer represented by Formula (v), a compound is preferable in which R¹¹ is a hydrogen atom or a methyl group, L¹ is an alkylene group, Z₁ is a carboxylic acid group, and Y is a methine group.

Furthermore, as the monomer represented by Formula (vi), a compound is preferable in which R¹⁴, R¹⁵, and R¹⁶ each independently represent a hydrogen atom or a methyl group, and Z₁ is a carboxylic acid group.

Typical examples of the monomers (compounds) represented by Formulas (iv) to (vi) will be shown below.

Examples of the monomers include methacrylic acid, crotonic acid, isocrotonic acid, a reactant of a compound containing an addition-polymerizable double bond and a hydroxyl group in a molecule (for example, 2-hydroxyethyl methacrylate) and a succinic anhydride, a reactant of a compound containing an addition-polymerizable double bond and a hydroxyl group in a molecule and a phthalic anhydride, a reactant of a compound containing an addition-polymerizable double bond and a hydroxyl group in a molecule and a tetrahydroxyphthalic anhydride, a reactant of a compound containing an addition-polymerizable double bond and a hydroxyl group in a molecule and a trimellitic anhydride, a reactant of a compound containing an addition-polymerizable double bond and a hydroxyl group in a molecule and a pyromellitic anhydride, acrylic acid, an acrylic acid dimer, an acrylic acid oligomer, maleic acid, itaconic acid, fumaric acid, 4-vinylbenzoic acid, vinylphenol, 4-hydroxyphenyl methacrylamide, and the like.

In view of interaction with the specific magnetic particles, temporal stability, and permeability with respect to a developer, the content of the repeating unit containing a functional group capable of interacting with the specific magnetic particles, the content being expressed in terms of mass, with respect to the total mass of the resin A is preferably 0.05% to 90% by mass, more preferably 1.0% to 80% by mass, and even more preferably 10% to 70% by mass.

### (Ethylenically unsaturated group)

The resin A may contain an ethylenically unsaturated group.

The ethylenically unsaturated group is not particularly limited, and examples thereof include a (meth)acryloyl group, a vinyl group, a styryl group, and the like. Among these, a (meth)acryloyl group is preferable.

Particularly, the resin A preferably contains a repeating unit that contains an ethylenically unsaturated group on a side chain, and more preferably contains a repeating unit that contains an ethylenically unsaturated group on a side chain and is derived from (meth)acrylate (hereinafter, such a repeating unit will be also called "(meth)acrylic repeating unit containing an ethylenically unsaturated group on a side chain").

The (meth)acrylic repeating unit containing an ethylenically unsaturated group on a side chain is obtained, for example, by causing an addition reaction between a carboxylic acid group in the resin A containing a (meth)acrylic repeating unit containing the carboxylic acid group and an ethylenically unsaturated compound containing a glycidyl group or an alicyclic epoxy group. In this way, a (meth)acrylic repeating unit containing an ethylenically unsaturated group on a side chain can be formed.

In a case where the resin A contains the repeating unit containing an ethylenically unsaturated group, the content of the repeating unit expressed in terms of mass with respect to the total mass of the resin A is preferably 30% to 70% by mass, and more preferably 40% to 60% by mass.

### (Other curable groups)

The resin A may contain other curable groups in addition to the ethylenically unsaturated group.

Examples of those other curable groups include an epoxy group and an oxetanyl group.

Particularly, the resin A preferably contains a repeating unit that contains those other curable groups on a side chain, and more preferably contains a repeating unit that contains those other curable groups on a side chain and is derived from (meth)acrylate (hereinafter, such a repeating unit will be also called "(meth)acrylic repeating unit containing other curable groups on a side chain").

Examples of the (meth)acrylic repeating unit containing other curable groups on a side chain include glycidyl (meth)acrylate.

In a case where the resin A contains the repeating unit containing other curable groups, the content of the repeating unit expressed in terms of mass with respect to the total mass of the resin A is preferably 5% to 50% by mass, and more preferably 10% to 30% by mass.

### (Other repeating units)

For the purpose of improving various performances such as film forming performance, as long as the effects of the present invention are not impaired, the resin A may further have other repeating units having various functions different from the repeating unit described above.

Examples of those other repeating units include repeating units derived from radically polymerizable compounds selected from acrylonitriles, methacrylonitriles, and the like.

For the resin A, one kind of those other repeating units or two or more kinds of those other repeating units can be used. The content of those other repeating units expressed in terms of mass with respect to the total mass of the resin A is preferably 0% to 80% by mass, and more preferably 10% to 60% by mass.

### (Physical properties of resin A)

The acid value of the resin A is not particularly limited. For example, the acid value is preferably 0 to 400 mgKOH/g, more preferably 10 to 350 mgKOH/g, even more preferably 30 to 300 mgKOH/g, and particularly preferably in a range of 50 to 200 mgKOH/g.

In a case where the acid value of the resin A is 50 mgKOH/g or more, the sedimentation stability of the specific magnetic particles can be further improved.

In the present specification, the acid value can be calculated, for example, from the average content of acid groups in a compound. Furthermore, changing the content of the repeating unit containing an acid group in the resin makes it possible to obtain a resin having a desired acid value.

The weight-average molecular weight of the resin A is not particularly limited. For example, the weight-average molecular weight is preferably 3,000 or more, more preferably 4,000 or more, even more preferably 5,000 or more, and particularly preferably 6,000 or more. The upper limit of the weight-average molecular weight is, for example, preferably 300,000 or less, more preferably 200,000 or less, even more preferably 100,000 or less, and particularly preferably 50,000 or less.

The resin A can be synthesized based on a known method.

For specific examples of the resin A, the polymer compounds described in paragraphs "0127" to "0129" of JP2013-249417A can be referred to, and what are described in the paragraphs are incorporated into the present specification.

As the resin A, the graft copolymers in paragraphs "0037" to "0115" of JP2010-106268A (paragraphs "0075" to "0133" of US2011/0124824 corresponding to JP2010-106268A) can also be used, and what are described in the paragraphs can be cited and incorporated into the present specification.

### <Alkali-soluble resin>

Those other resins may include an alkali-soluble resin.

In the present specification, the alkali-soluble resin means a resin that contains a group (alkali-soluble group, for example, an acid group such as a carboxylic acid group) enhancing alkali solubility and is different from the resin A described above.

Examples of the alkali-soluble resin include a resin containing at least one alkali-soluble group in a molecule. Examples thereof include a polyhydroxystyrene resin, a polysiloxane resin, a (meth)acrylic resin, a (meth)acrylamide resin, a (meth)acrylic/(meth)acrylamide copolymer, an epoxy resin, a polyimide resin, and the like.

Specific examples of the alkali-soluble resin include a copolymer of an unsaturated carboxylic acid and an ethylenically unsaturated compound.

The unsaturated carboxylic acid is not particularly limited, and examples thereof include monocarboxylic acid such as (meth)acrylic acid, crotonic acid, and vinylacetic acid; dicarboxylic acids such as itaconic acid, maleic acid, and fumaric acid or anhydrides of these acids; polyvalent carboxylic acid monoesters such as mono(2-(meth)acryloyloxyethyl)phthalate; and the like.

Examples of copolymerizable ethylenically unsaturated compounds include methyl (meth)acrylate and the like. Furthermore, the compounds described in paragraphs "0027" of JP2010-097210A and paragraphs "0036" and "0037" of JP2015-068893A can also be used, and what are described in the above paragraphs are incorporated into the present specification.

Furthermore, a compound that is a copolymerizable ethylenically unsaturated compound and contains an ethylenically unsaturated group on a side chain may also be used in combination. That is, the alkali-soluble resin may contain a repeating unit containing an ethylenically unsaturated group on a side chain.

As the ethylenically unsaturated group contained on a side chain, a (meth)acrylic acid group is preferable.

The repeating unit containing an ethylenically unsaturated group on a side chain is obtained, for example, by causing an addition reaction between a carboxylic acid group of a (meth)acrylic repeating unit containing the carboxylic acid group and an ethylenically unsaturated compound containing a glycidyl group or an alicyclic epoxy group.

As the alkali-soluble resin, an alkali-soluble resin containing a curable group is also preferable.

Examples of the curable group include an ethylenically unsaturated group (for example, a (meth)acryloyl group, a vinyl group, a styryl group, or the like), a cyclic ether group (for example, an epoxy group, an oxetanyl group, or the like), and the like. However, the curable group is not limited to these.

As the curable group, among these, in view of making it possible to control polymerization by a radical reaction, an ethylenically unsaturated group is preferable, and a (meth)acryloyl group is more preferable.

As the alkali-soluble resin containing a curable group, an alkali-soluble resin having a curable group on a side chain or the like is preferable. Examples of the alkali-soluble resin containing a curable group include DIANAL NR series (manufactured by MITSUBISHI RAYON CO., LTD.), Photomer 6173 (COOH-containing polyurethane acrylic oligomer, manufactured by Diamond Shamrock Co., Ltd.), VISCOAT R-264 and KS Resist 106 (all are manufactured by OSAKA ORGANIC CHEMICAL INDUSTRY LTD.), CYCLOMER P series (for example, ACA230AA) and PLACCEL CF200 series (all are manufactured by Daicel Corporation), Ebecryl 3800 (manufactured by DAICEL-ALLNEX LTD.), and ACRYCURE RD-F8 (manufactured by NIPPON SHOKUBAI CO., LTD.), and the like.

As the alkali-soluble resin, for example, it is possible to use a radical polymer containing a carboxylic acid group on a side chain described in JP1984-044615A (JP-S59-044615A), JP1979-034327B (JP-S54-034327AB), JP1983-12577B (JP-S58-12577B), JP1979-25957B (JP-S54-25957B), JP1979-92723B (JP-S54-92723B), JP1984-053836A (JP-S59-053836A), and JP1984-071048A (JP-S59-071048A); an acetal-modified polyvinyl alcohol-based binder resin containing an alkali-soluble group described in EP993966B, EP1204000B, and JP2001-318463A; polyvinylpyrrolidone; polyethylene oxide; alcohol-soluble nylon, polyether as a reactant of 2,2-bis-(4-hydroxyphenyl)-propane and epichlorohydrin, and the like; the polyimide resin described WO2008/123097A; and the like.

As the alkali-soluble resin, for example, the compounds described in paragraphs "0225" to "0245" of JP2016-075845A can also be used, and what are described in the above paragraphs are incorporated into the present specification.

As the alkali-soluble resin, a polyimide precursor can also be used. The polyimide precursor means a resin obtained by causing an addition polymerization reaction between a compound containing an acid anhydride group and a diamine compound at 40°C to 100°C.

Specific examples of the polyimide precursor include the compounds described in paragraphs "0011" to "0031" of JP2008-106250A, the compounds described in paragraphs "0022" to "0039" of JP2016-122101A, the compounds described in paragraphs "0061" to "0092" of JP2016-068401A, the resins described in paragraph "0050" of JP2014-137523A, the resins described in paragraph "0058" of JP2015-187676A, the resins described in paragraphs "0012" and "0013" of JP2014-106326A, and the like. What are described in the above paragraphs are incorporated into the present specification.

As the alkali-soluble resin, a [benzyl (meth)acrylate/(meth)acrylic acid/other addition-polymerizable vinyl monomers used as necessary] copolymer and an [allyl(meth)acrylate/(meth)acrylic acid/other addition-polymerizable vinyl monomers used as necessary] copolymer are suitable because these make film hardness, sensitivity, and developability well balanced.

One of the aforementioned other addition-polymerizable vinyl monomers may be used alone, or two or more of such monomers may be used in combination.

In view of further improving moisture resistance of a cured film, the aforementioned copolymers preferably have a curable group, and more preferably have an ethylenically unsaturated group such as a (meth)acryloyl group.

For example, monomers have a curable group may be used as the aforementioned other addition-polymerizable vinyl monomers such that the curable group is introduced into the copolymers. In addition, a curable group (preferably an ethylenically unsaturated group such as a (meth)acryloyl group) may be introduced into some or all of one or more units derived from (meth)acrylic acid and/or one or more units derived from the aforementioned other addition-polymerizable vinyl monomers in the copolymers.

Examples of the aforementioned other addition-polymerizable vinyl monomers include methyl (meth)acrylate, a styrene-based monomer (such as hydroxystyrene), and an ether dimer.

Examples of the ether dimer include a compound represented by the following General Formula (ED1) and a compound represented by the following General Formula (ED2).

In General Formula (ED1), R¹ and R² each independently represent a hydrogen atom or a hydrocarbon group with a carbon number of 1 to 25.

In General Formula (ED2), R represents a hydrogen atom or an organic group with a carbon number of 1 to 30. For specific examples of General Formula (ED2), the description of JP2010-168539A can be referred to.

For specific examples of the ether dimer, for example, paragraph "0317" of JP2013-029760A can be referred to, and what are described in the paragraph are incorporated into the present specification. Only one ether dimer may be used alone, or two or more ether dimers may be used.

The acid value of the alkali-soluble resin is not particularly limited. Generally, the acid value is preferably 30 to 500 mgKOH/g, and more preferably 50 to 200 mgKOH/g or more.

In a case where the composition contains an alkali-soluble resin, the content of the alkali-soluble resin with respect to the total mass of the composition is preferably 0.1% to 40% by mass, more preferably 0.5% to 30% by mass, and even more preferably 1% to 20% by mass.

In a case where the composition contains an alkali-soluble resin, the content of the alkali-soluble resin with respect to the total solid content of the composition is preferably 0.1% to 40% by mass, more preferably 0.5% to 30% by mass, and even more preferably 1% to 20% by mass.

### [Polymerizable Compound]

The composition according to the embodiment of the present invention may contain a polymerizable compound as a component different from the components described above.

The content of the polymerizable compound with respect to the total mass of the composition is preferably 1% to 35% by mass, more preferably 1% to 30% by mass, and even more preferably 3% to 27% by mass.

The content of the polymerizable compound with respect to the total solid content of the composition is preferably 1% to 35% by mass, more preferably 1% to 30% by mass, and even more preferably 3% to 27% by mass.

The molecular weight (or weight-average molecular weight) of the polymerizable compound is not particularly limited, but is preferably 2,000 or less.

### <Compound containing group containing ethylenically unsaturated bond>

Examples of an aspect of the polymerizable compound include a compound containing a group containing an ethylenically unsaturated bond (hereinafter, also simply called "ethylenically unsaturated group").

That is, it is preferable that in an aspect, the composition according to the embodiment of the present invention contain, as a polymerizable compound, a low-molecular-weight compound containing an ethylenically unsaturated group.

The polymerizable compound is preferably a compound containing one or more ethylenically unsaturated bonds, more preferably a compound containing two or more ethylenically unsaturated bonds, even more preferably a compound containing three or more ethylenically unsaturated bonds, and particularly preferably a compound containing five or more ethylenically unsaturated bonds. The upper limit of the number of ethylenically unsaturated bonds is, for example, 15 or less. Examples of the ethylenically unsaturated group include a vinyl group, a (meth)allyl group, a (meth)acryloyl group, and the like.

As the polymerizable compound, for example, it is possible to use the compounds described in paragraph "0050" of JP2008-260927A and paragraph "0040" of JP2015-068893A, and what are described in the paragraphs are incorporated into the present specification.

The polymerizable compound may be in any chemical form such as a monomer, a prepolymer, an oligomer, a mixture of these, and a multimer of these.

The polymerizable compound is preferably a (meth)acrylate compound having 3 to 15 functional groups, and more preferably a (meth)acrylate compound having 3 to 6 functional groups.

As the polymerizable compound, a compound that contains one or more ethylenically unsaturated groups and has a boiling point of 100°C or higher under normal pressure is also preferable. For example, the compounds described in paragraph "0227" of JP2013-029760A and paragraph "0254" to "0257" of JP2008-292970A can be referred to, and what are described in the paragraphs are incorporated into the present specification.

As the polymerizable compound, dipentaerythritol triacrylate (KAYARAD D-330 as a commercially available product; manufactured by Nippon Kayaku Co., Ltd.), dipentaerythritol tetraacrylate (KAYARAD D-320 as a commercially available product; manufactured by Nippon Kayaku Co., Ltd.), dipentaerythritol penta(meth)acrylate (KAYARAD D-310 as a commercially available product; manufactured by Nippon Kayaku Co., Ltd.), dipentaerythritol hexa(meth)acrylate (KAYARAD DPHA as a commercially available product; manufactured by Nippon Kayaku Co., Ltd., A-DPH-12E; manufactured by SHIN-NAKAMURA CHEMICAL CO, LTD.), and the structure in which these (meth)acryloyl groups are mediated by an ethylene glycol residue or a propylene glycol residue (for example, SR454 and SR499 commercially available from Sartomer Company Inc.) are preferable. These compounds in oligomer types can also be used. Furthermore, NK ESTER A-TMMT (pentaerythritol tetraacrylate, manufactured by SHIN-NAKAMURA CHEMICAL CO, LTD.), A-TMMT (polyfunctional acrylate, manufactured by TOAGOSEI CO., LTD.), KAYARAD RP-1040, KAYARAD DPEA-12LT, KAYARAD DPHA LT, KAYARAD RP-3060, and KAYARAD DPEA-12 (all are trade names, manufactured by Nippon Kayaku Co., Ltd.), and the like may also be used.

The polymerizable compound may have an acid group such as a carboxylic acid group, a sulfonic acid group, or a phosphoric acid group. The polymerizable compound containing an acid group is preferably an ester of an aliphatic polyhydroxy compound and an unsaturated carboxylic acid, more preferably a polymerizable compound obtained by reacting an unreacted hydroxyl group of an aliphatic polyhydroxy compound with a non-aromatic carboxylic anhydride such that an acid group is added, and even more preferably an ester of the aforementioned polymerizable compound having pentaerythritol and/or dipentaerythritol as the aliphatic polyhydroxy compound. Examples of commercially available products thereof include ARONIX TO-2349, M-305, M-510, and M-520 manufactured by TOAGOSEI CO., LTD., and the like.

The acid value of the polymerizable compound containing an acid group is preferably 0.1 to 40 mgKOH/g, and more preferably 5 to 30 mgKOH/g. In a case where the acid value of the polymerizable compound is 0.1 mgKOH/g or more, development and dissolution characteristics are excellent. In a case where the acid value is 40 mgKOH/g or less, this is advantageous in terms of manufacturing and/or handling. Furthermore, excellent photopolymerization performance and excellent curing properties are obtained.

As the polymerizable compound, a compound containing a caprolactone structure is also a preferred aspect.

The compound containing a caprolactone structure is not particularly limited as long as the compound contains the caprolactone structure in a molecule. Examples thereof include ε-caprolactone-modified polyfunctional (meth)acrylate obtained by esterifying a polyhydric alcohol, such as trimethylolethane, ditrimethylolethane, trimethylolpropane, ditrimethylolpropane, pentaerythritol, dipentaerythritol, tripentaerythritol, glycerin, diglycerol, or trimethylol melamine, (meth)acrylic acid, and ε-caprolactone. Among these, a compound containing a caprolactone structure represented by the following Formula (Z-1) is preferable.

In Formula (Z-1), all six Rs are groups represented by the following Formula (Z-2), or one to five out of six Rs are groups represented by the following Formula (Z-2) and others are groups represented by the following Formula (Z-3).

In Formula (Z-2), R¹ represents a hydrogen atom or a methyl group, m represents a number of 1 or 2, and "*" represents a bonding site.

In Formula (Z-3), R¹ represents a hydrogen atom or a methyl group, and "*" represents a bonding site.

The polymerizable compound containing a caprolactone structure is commercially available from Nippon Kayaku Co., Ltd., for example, as KAYARAD DPCA series. Examples thereof include DPCA-20 (compound where m in the above Formulas (Z-1) to (Z-3) is 1, the number of groups represented by Formula (Z-2) is 2, and R¹'s all represent a hydrogen atom), DPCA-30 (compound where m in the above Formulas (Z-1) to (Z-3) is 1, the number of groups represented by Formula (Z-2) is 3, and R¹'s all represent a hydrogen atom), DPCA-60 (compound where m in the above Formulas (Z-1) to (Z-3) is 1, the number of groups represented by Formula (Z-2) is 6, and R¹'s all represent a hydrogen atom), DPCA-120 (compound where m in the above Formulas (Z-1) to (Z-3) is 2, the number of groups represented by Formula (Z-2) is 6, and R¹'s all represent a hydrogen atom), and the like. Furthermore, examples of commercially available products of the polymerizable compound containing a caprolactone structure include M-350 (trade name) (trimethylolpropane triacrylate) manufactured by TOAGOSEI CO., LTD.

As the polymerizable compound, a compound represented by the following Formula (Z-4) or (Z-5) can also be used.

In Formulas (Z-4) and (Z-5), E represents-((CH₂)_{y}CH₂O)- or ((CH₂)_{y}CH(CH₃)O)-, y represents an integer of 0 to 10, and X represents a (meth)acryloyl group, a hydrogen atom, or a carboxylic acid group.

In Formula (Z-4), the total number of (meth)acryloyl groups is 3 or 4, m represents an integer of 0 to 10, and the total of m's is an integer of 0 to 40.

In Formula (Z-5), the total number of (meth)acryloyl groups is 5 or 6, n represents an integer of 0 to 10, and the total of n's is an integer of 0 to 60.

In Formula (Z-4), m is preferably an integer of 0 to 6, and more preferably an integer of 0 to 4.

The total of m's is preferably an integer of 2 to 40, more preferably an integer of 2 to 16, and even more preferably an integer of 4 to 8.

In Formula (Z-5), n is preferably an integer of 0 to 6, and more preferably an integer of 0 to 4.

The total of n's is preferably an integer of 3 to 60, more preferably an integer of 3 to 24, and even more preferably an integer of 6 to 12.

In addition, as for -((CH₂)_{y}CH₂O)- or ((CH₂)_{y}CH(CH₃)O)- in Formula (Z-4) or Formula (Z-5), it is preferable that the terminal on the oxygen atom side be bonded to X.

One compound represented by Formula (Z-4) or Formula (Z-5) may be used alone, or two or more such compounds may be used in combination. Especially, it is preferable to employ an aspect in which all of six Xs in Formula (Z-5) represent an acryloyl group or an aspect in which a compound represented by Formula (Z-5) where all of six Xs represent an acryloyl group and a compound represented by Formula (Z-5) where at least one of six Xs represents a hydrogen atom form a mixture. This constitution can further improve developability.

The total content of the compound represented by Formula (Z-4) or Formula (Z-5) in the polymerizable compound is preferably 20% by mass or more, and more preferably 50% by mass or more.

Among the compounds represented by Formula (Z-4) or Formula (Z-5), either or both of a pentaerythritol derivative and a dipentaerythritol derivative are more preferable.

The polymerizable compound may contain a cardo skeleton.

As the polymerizable compound containing a cardo skeleton, a polymerizable compound containing a 9,9-bisarylfluorene skeleton is preferable.

Examples of the polymerizable compound containing a cardo skeleton include, but are not limited to, ONCOAT EX series (manufactured by NAGASE & CO., LTD.), OGSOL (manufactured by Osaka Gas Chemicals Co., Ltd.), and the like.

As the polymerizable compound, a compound containing an isocyanuric acid skeleton as a core is also preferable. Examples of such a polymerizable compound include NK ESTER A-9300 (manufactured by SHIN-NAKAMURA CHEMICAL CO, LTD.).

The content of ethylenically unsaturated groups in the polymerizable compound (the content means a value obtained by dividing the number of ethylenically unsaturated groups in the polymerizable compound by the molecular weight (g/mol) of the polymerizable compound) is preferably 5.0 mmol/g or more. The upper limit of the content is not particularly limited, but is generally 20.0 mmol/g or less.

### <Compound containing one or more epoxy groups and one or more oxetanyl groups>

Examples of one aspect of the polymerizable compound include a compound containing one or more epoxy groups and one or more oxetanyl groups.

That is, in one aspect, it is preferable that the composition according to the embodiment of the present invention contain, as a polymerizable compound, a compound containing one or more epoxy groups and one or more oxetanyl groups.

The polymerizable compound is preferably a compound containing one or more epoxy groups and/or one or more oxetanyl groups, and more preferably a compound containing two or more epoxy groups and/or two or more oxetanyl groups. The upper limit of the number of epoxy groups and/or oxetanyl groups is, for example, 10 or less.

Particularly, the polymerizable compound is more preferably curable epoxy compound having an epoxy group (epoxy compound).

In the polymerizable compound, the epoxy group and/or oxetanyl group (preferably epoxy group) may be fused with a cyclic group (such as an alicyclic group). The cyclic group fused with an epoxy group and/or an oxetanyl group preferably has a carbon number of 5 to 15. In addition, in the above cyclic group, the portion other than the fused epoxy group and/or oxetanyl group may be monocyclic or polycyclic. One cyclic group may be fused with only one epoxy group or oxetanyl group, or may be fused with two or more epoxy groups and/or oxetanyl groups.

Examples of such a polymerizable compound include a monofunctional or polyfunctional glycidyl ether compound.

The polymerizable compound may be, for example, (poly)alkylene glycol diglycidyl ether.

The polymerizable compound may be a compound containing a caprolactone structure represented by Formula (Z-1) described above in which the group represented by Formula (Z-2) is changed to the following Formula (Z-2E) and the group represented by Formula (Z-3) is changed to a group represented by Formula (Z-3E).

In Formula (Z-2E), m represents the number 1 or 2, X and Y each independently represent a hydrogen atom or a substituent (preferably an alkyl group preferably having a carbon number of 1 to 3), and "*" represents a bonding site.

In Formula (Z-3E), X and Y each independently represent a hydrogen atom or a substituent (preferably an alkyl group preferably having a carbon number of 1 to 3), and "*" represents a bonding site.

The polymerizable compound may be a compound represented by Formula (Z-4) described above in which X is changed to represent a group represented by Formula (Z-3E) or a hydrogen atom.

In Formula (Z-4) modified in this way, the total number of groups represented by formula (Z-3E) is 2 to 4.

The polymerizable compound may be a compound represented by Formula (Z-5) described above in which X is changed to represent a group represented by Formula (Z-3E) or a hydrogen atom.

In Formula (Z-5) modified in this way, the total number of groups represented by Formula (Z-3E) is 2 to 6 (preferably 5 or 6).

The polymerizable compound may be a compound having a structure to which N pieces of cyclic groups fused with an epoxy group and/or an oxetanyl group are bonded via a linking group.

N is an integer of 2 or more, preferably an integer of 2 to 6, and more preferably 2. In the linking group, the total number of atoms other than hydrogen atoms is preferably 1 to 20 and more preferably 2 to 6. In a case where N is 2, examples of the linking group include an alkyleneoxycarbonyl group.

Examples of commercially available products of the polymerizable compound include polyfunctional aliphatic glycidyl ether compounds such as DENACOL EX-212L, EX-214L, EX-216L, EX-321L, and EX-850L (all are manufactured by Nagase ChemteX Corporation.). Although these are low-chlorine products, EX-212, EX-214, EX-216, EX-321, EX-614, EX-850, and the like that are not low-chlorine products can also be used.

Furthermore, as a commercially available product, CELLOXIDE 2021P (manufactured by Daicel Corporation, a polyfunctional epoxy monomer) can also be used.

The composition may contain, as polymerizable compounds, both the compound containing a group containing an ethylenically unsaturated bond and a compound containing one or more epoxy groups and one or more oxetanyl groups. In this case, the mass ratio of the contents thereof (content of "compound containing a group containing an ethylenically unsaturated bond"/content of "compound containing either or both of an epoxy group and an oxetanyl group") is preferably 10/90 to 90/10, more preferably 20/80 to 80/20, and even more preferably 30/70 to 70/30.

### [Curing accelerator]

The composition may contain a curing accelerator.

Particularly, in a case where the composition contains a compound having an epoxy group and/or an oxetanyl group as a polymerizable compound, it is preferable that the composition contain a curing accelerator.

Examples of the curing accelerator include triphenylphosphine, methyltributylphosphonium dimethylphosphate, trisorthotolylphosphine, and a boron trifluoride amine complex. Examples of the curing accelerator also include imidazole-based curing accelerators such as 2-methylimidazole (trade name; 2MZ), 2-undecylimidazole (trade name; C11-Z), 2-heptadecylimidazole (trade name; C17Z), 1,2-dimethylimidazole (trade name; 1.2 DMZ), 2-ethyl-4-methylimidazole (trade name; 2E4MZ), 2-phenylimidazole (trade name; 2PZ), 2-phenyl-4-methylimidazole (trade name; 2P4MZ), 1-benzyl-2-methylimidazole (trade name; 1B2MZ), 1-benzyl-2-phenylimidazole (trade name; 1B2PZ), 1-cyanoethyl-2-methylimidazole (trade name; 2MZ-CN), 1-cyanoethyl-2- undecylimidazole (trade name; C11Z-CN), 1-cyanoethyl-2-phenylimidazolium trimellitate (trade name; 2PZCNS-PW), 2,4-diamino-6-[2'-methylimidazolyl-(1')]-ethyl-s-triazine (trade name; 2MZ-A), 2,4-diamino-6-[2'-undecylimidazolyl-(1')]-ethyl-s-triazine (trade name; C11Z-A), 2,4-diamino-6-[2'-ethyl-4'-methylimidazolyl-(1')]-ethyl-s-triazine (trade name; 2E4MZ-A), 2,4-diamino-6-[2'-methylimidazolyl-(1')]-ethyl-s-triazine isocyanuric acid adduct (trade name; 2MA-OK), 2-phenyl-4,5-dihydroxymethylimidazole (trade name; 2PHZ-PW), 2-phenyl-4-methyl-5-hydroxymethylimidazole (trade name; 2P4MHZ-PW), 1-cyanoethyl-2-phenylimidazole (trade name; 2PZ-CN), 2,4-diamino-6-[2'-methylimidazolyl-(1')]-ethyl-s-triazine (trade name; 2MZA-PW), and 2,4-diamino-6-[2'-methylimidazolyl-(1')]-ethyl-s-triazine isocyanuric acid adduct(trade name: 2MAOK-PW) (all manufactured by SHIKOKU CHEMICALS CORPORATION.) Examples of triarylphosphine-based curing accelerators also include the compounds described in paragraph "0052" of JP2004-043405A. Examples of the phosphorus-based curing accelerators in which triphenylborane is added to triarylphosphine include the compounds described in paragraph "0024" of JP2014-005382A.

The content of the curing accelerator with respect to the total mass of the composition is preferably 0.0002% to 3% by mass, more preferably 0.002% to 2% by mass, and even more preferably 0.02% to 1% by mass.

The content of the curing accelerator with respect to the total solid content of the composition is preferably 0.0002% to 3% by mass, more preferably 0.002% to 2% by mass, and even more preferably 0.02% to 1% by mass.

### [Polymerization Initiator]

The composition may contain a polymerization initiator.

As the polymerization initiator, known polymerization initiators can be used without particular limitation. Examples of the polymerization initiator include a photopolymerization initiator, a thermal polymerization initiator, and the like. Among these, a photopolymerization initiator is preferable. As the polymerization initiator, a so-called radical polymerization initiator is preferable.

In a case where the composition contains a polymerization initiator, the content of the polymerization initiator with respect to the total mass of the composition is preferably 0.3% to 15% by mass, more preferably 0.3% to 10% by mass, and even more preferably 0.3% to 8.0% by mass.

In a case where the composition contains a polymerization initiator, the content of the polymerization initiator with respect to the total solid content of the composition is preferably 0.3% to 15% by mass, more preferably 0.3% to 10% by mass, and even more preferably 0.3% to 8.0% by mass.

### <Thermal polymerization initiator>

Examples of the thermal polymerization initiator include azo compounds such as 2,2'-azobisisobutyronitrile (AIBN), 3-carboxypropionitrile, azobismalenonitrile, and dimethyl-(2,2')-azobis(2-methylpropionate) [V-601] and organic peroxides such as benzoyl peroxide, lauroyl peroxide, and potassium persulfate.

Specific examples of the polymerization initiator include the polymerization initiators described on pages 65 to 148 of "Ultraviolet Curing System" by Kiyomi Kato (published by GL Sciences Inc.: 1989), and the like.

### <Photopolymerization Initiator>

The photopolymerization initiator is not particularly limited as long as it can initiate the polymerization of the polymerizable compound. As the photopolymerization initiator, known photopolymerization initiators can be used. As the photopolymerization initiator, for example, a photopolymerization initiator sensitive to light ranging from an ultraviolet region to a visible light region is preferable. Furthermore, the photopolymerization initiator may be an activator that brings a certain action together with a photoexcited sensitizer and generates active radicals or an initiator that initiates cationic polymerization according to the type of polymerizable compound.

In addition, it is preferable that the photopolymerization initiator contain at least one compound having molar absorption coefficient of at least 50 in a range of 300 to 800 nm (more preferably 330 to 500 nm).

Examples of the photopolymerization initiator include halogenated hydrocarbon derivatives (for example, a compound containing a triazine skeleton, a compound containing an oxadiazole skeleton, and the like), acylphosphine compounds such as acylphosphine oxide, hexaarylbiimidazole, oxime compounds such as oxime derivatives, organic peroxides, thio compounds, ketone compounds, aromatic onium salts, aminoacetophenone compounds, hydroxyacetophenone, and the like.

For specific examples of the photopolymerization initiator, for example, paragraphs "0265" to "0268" of JP2013-029760A can be referred to, and what are described in the paragraphs are incorporated into the present specification.

More specifically, as the photopolymerization initiator, for example, the aminoacetophenone-based initiator described in JP1998-291969A (JP-H10-291969A) and the acylphosphine-based initiator described in JP4225898B can also be used.

As hydroxyacetophenone compounds, for example, Omnirad-184, Omnirad-1173, Omnirad-500, Omnirad-2959, and Omnirad-127 (trade names, all manufactured by IGM Resins B.V) can be used.

As aminoacetophenone compounds, for example, commercially available products, Omnirad-907, Omnirad-369, and Omnirad-379EG (trade names, all manufactured by IGM Resins B.V), can be used. As aminoacetophenone compounds, it is also possible to use the compound described in JP2009-191179A having an absorption wavelength matched with a long wavelength light source having a wavelength of 365 nm or a wavelength of 405 nm.

As acylphosphine compounds, for example, commercially available products, Omnirad-819 and Omnirad-TPO (trade names, all manufactured by IGM Resins B.V), can be used.

As the photopolymerization initiator, an oxime ester-based polymerization initiator (oxime compound) is more preferable. Particularly, an oxime compound is preferable because this compound has high sensitivity and high polymerization efficiency and makes it easy to design a high coloring material content in the composition.

Specifically, as the oxime compound, for example, the compound described in JP2001-233842A, the compound described in JP2000-80068A, or the compound described in JP2006-342166A can be used.

Examples of the oxime compound include 3-benzoyloxyiminobutan-2-one, 3-acetoxyiminobutan-2-one, 3-propionyloxyiminobutan-2-one, 2-acetoxyiminopentan-3-one, 2-acetoxyimino-1-phenylpropan-1-one, 2-benzoyloxyimino-1-phenylpropan-1-one, 3-(4-toluenesulfonyloxy)iminobutan-2-one, 2-ethoxycarbonyloxyimino-1-phenylpropan-1-one, and the like.

Examples of the oxime compound also include the compounds described in J. C. S. Perkin II (1979) pp. 1653-1660, J. C. S. Perkin II (1979) pp. 156-162, Journal of Photopolymer Science and Technology (1995) pp. 202-232, and JP2000-066385A, the compounds described in JP2000-080068A, JP2004-534797A, and JP2006-342166A, and the like.

As commercially available products, IRGACURE-OXE01 (manufactured by BASF SE), IRGACURE-OXE02 (manufactured by BASF SE), IRGACURE-OXE03 (manufactured by BASF SE), or IRGACURE-OXE04 (manufactured by BASF SE) is also preferable. In addition, TR-PBG-304 (manufactured by Changzhou Tronly New Electronic Materials Co., Ltd.), ADEKA ARKLS NCI-831 and ADEKA ARKLS NCI-930 (manufactured by ADEKA CORPORATION), or N-1919 (carbazole oxime ester skeleton-containing photoinitiator (manufactured by ADEKA CORPORATION)) can also be used.

Furthermore, as oxime compounds other than the above, the compound described in JP2009-519904A in which oxime is linked to the N-position of carbazole; the compound described in US7626957B in which a hetero substituent is introduced into a benzophenone moiety; the compounds described in JP2010-015025A and US2009-292039A in which a nitro group is introduced into a dye moiety; the ketoxime compound described in WO2009-131189A; the compound described in US7556910B that contains a triazine skeleton and an oxime skeleton in the same molecule; the compound described in JP2009-221114A that has absorption maximum at 405 nm and has excellent sensitivity to a g-line light source; and the like may also be used.

For example, paragraphs "0274" and "0275" of JP2013-029760A can be referred to, and what are described in the paragraphs are incorporated into the present specification.

Specifically, as the oxime compound, a compound represented by the following Formula (OX-1) is preferable. The aforementioned oxime compound may be an oxime compound in which the N-O bond is an (E) isomer, an oxime compound in which the N-O bond is a (Z) isomer, or an oxime compound in which the N-O bond is a mixture of an (E) isomer and a (Z) isomer.

In Formula (OX-1), R and B each independently represent a monovalent substituent, A represents a divalent organic group, and Ar represents an aryl group.

In Formula (OX-1), as the monovalent substituent represented by R, a monovalent non-metal atomic group is preferable.

Examples of the monovalent non-metal atomic group include an alkyl group, an aryl group, an acyl group, an alkoxycarbonyl group, an aryloxycarbonyl group, a heterocyclic group, an alkylthiocarbonyl group, an arylthiocarbonyl group, and the like. Furthermore, these groups may have one or more substituents. In addition, the aforementioned substituents may be further substituted with another substituent.

Examples of the substituent include a halogen atom, an aryloxy group, an alkoxycarbonyl or aryloxycarbonyl group, an acyloxy group, an acyl group, an alkyl group, an aryl group, and the like.

As the monovalent substituent represented by B in Formula (OX-1), an aryl group, a heterocyclic group, an arylcarbonyl group, or a heterocyclic carbonyl group is preferable, and an aryl group or a heterocyclic group is more preferable. These groups may have one or more substituents. Examples of the substituents include the aforementioned substituents.

As the divalent organic group represented by A in Formula (OX-1), an alkylene group with a carbon number of 1 to 12, a cycloalkylene group, or an alkynylene group is preferable. These groups may have one or more substituents. Examples of the substituents include the aforementioned substituents.

As the photopolymerization initiator, an oxime compound containing a fluorine atom can also be used. Specific examples of the oxime compound containing a fluorine atom include the compounds described in JP2010-262028A; compounds 24 and 36 to 40 described in JP2014-500852A; the compound (C-3) described in JP2013-164471A; and the like. What are described in these documents are incorporated into the present specification.

As the photopolymerization initiator, compounds represented by the following Formulas (1) to (4) can also be used.

In Formula (1), R¹ and R² each independently represent an alkyl group with a carbon number of 1 to 20, an alicyclic hydrocarbon group with a carbon number of 4 to 20, an aryl group with a carbon number of 6 to 30, or an arylalkyl group with a carbon number of 7 to 30; in a case where R¹ and R² represent phenyl groups, the phenyl groups may be bonded together to form a fluorene group; R³ and R⁴ each independently represent a hydrogen atom, an alkyl group with a carbon number of 1 to 20, an aryl group with a carbon number of 6 to 30, an arylalkyl group with a carbon number of 7 to 30, or a heterocyclic group with a carbon number of 4 to 20; and X represents a direct bond or a carbonyl group.

In Formula (2), R¹, R², R³, and R⁴ have the same definitions as R¹, R², R³, and R⁴ in Formula (1), R⁵ represents -R⁶, -OR⁶, -SR⁶, -COR⁶, -CONR⁶R⁶, -NR⁶COR⁶, -OCOR⁶, -COOR⁶, -SCOR⁶, -OCSR⁶, -COSR⁶, -CSOR⁶, -CN, a halogen atom, or a hydroxyl group, R⁶ represents an alkyl group with a carbon number of 1 to 20, an aryl group with a carbon number of 6 to 30, an arylalkyl group with a carbon number of 7 to 30, or a heterocyclic group with a carbon number of 4 to 20, X represents a direct bond or a carbonyl group, and a represents an integer of 0 to 4.

In Formula (3), R¹ represents an alkyl group with a carbon number of 1 to 20, an alicyclic hydrocarbon group with a carbon number of 4 to 20, an aryl group with a carbon number of 6 to 30, or an arylalkyl group with a carbon number of 7 to 30; R³ and R⁴ each independently represent a hydrogen atom, an alkyl group with a carbon number of 1 to 20, an aryl group with a carbon number of 6 to 30, an arylalkyl group with a carbon number of 7 to 30, or a heterocyclic group with a carbon number of 4 to 20; and X represents a direct bond or a carbonyl group.

In Formula (4), R¹, R³, and R⁴ have the same definitions as R¹, R³, and R⁴ in Formula (3), R⁵ represents -R⁶, -OR⁶, -SR⁶, -COR⁶, -CONR⁶R⁶, -NR⁶COR⁶, -OCOR⁶, -COOR⁶, -SCOR⁶, -OCSR⁶, -COSR⁶, -CSOR⁶, -CN, a halogen atom, or a hydroxyl group, R⁶ represents an alkyl group with a carbon number of 1 to 20, an aryl group with a carbon number of 6 to 30, an arylalkyl group with a carbon number of 7 to 30, or a heterocyclic group with a carbon number of 4 to 20, X represents a direct bond or a carbonyl group, and a represents an integer of 0 to 4.

In the Formulas (1) and (2), each of R¹ and R² is preferably a methyl group, an ethyl group, an n-propyl group, an i-propyl group, a cyclohexyl group, or a phenyl group. R³ is preferably a methyl group, an ethyl group, a phenyl group, a tolyl group, or a xylyl group. R⁴ is preferably an alkyl group or a phenyl group with a carbon number of 1 to 6. R⁵ is preferably a methyl group, an ethyl group, a phenyl group, a tolyl group, or a naphthyl group. X is preferably a direct bond.

In the Formulas (3) and (4), R¹ is preferably a methyl group, an ethyl group, an n-propyl group, an i-propyl group, a cyclohexyl group, or a phenyl group. R³ is preferably a methyl group, an ethyl group, a phenyl group, a tolyl group, or a xylyl group. R⁴ is preferably an alkyl group with a carbon number of 1 to 6, or a phenyl group. R⁵ is preferably a methyl group, an ethyl group, a phenyl group, a tolyl group, or a naphthyl group. X is preferably a direct bond.

Specific examples of the compounds represented by Formulas (1) and (2) include the compounds described in paragraphs "0076" to "0079" of JP2014-137466A. What are described in these documents are incorporated into the present specification.

Specific examples of the oxime compound preferably used in the aforementioned composition will be shown below. Among the following oxime compounds, the oxime compound represented by General Formula (C-13) is more preferable.

Furthermore, as the oxime compound, the compounds described in Table 1 of WO2015/036910A can also be used, and what are described in the document are incorporated into the present specification.

The oxime compound preferably has a maximal absorption wavelength in a wavelength range of 350 to 500 nm, more preferably has a maximal absorption wavelength in a wavelength range of 360 to 480 nm, and even more preferably has a high absorbance at wavelengths of 365 nm and 405 nm.

In view of sensitivity, the molar absorption coefficient of the oxime compound at 365 nm or 405 nm is preferably 1,000 to 300,000, more preferably 2,000 to 300,000, and even more preferably 5,000 to 200,000.

The molar absorption coefficient of a compound can be measured using known methods. For example, it is preferable to measure the molar absorption coefficient by using an ultraviolet-visible spectrophotometer (Cary-5 spectrophotometer manufactured by Varian) and ethyl acetate at a concentration of 0.01 g/L.

As necessary, two or more photopolymerization initiators may be used in combination.

As the photopolymerization initiator, it is also possible to use the compounds described in paragraph "0052" of JP2008-260927A, paragraphs "0033" to 0037 of JP2010-97210A, and paragraph "0044" of JP2015-068893A, and what are described in the paragraphs are incorporated into the present specification. In addition, the oxime initiator described in KR10-2016-0109444A can also be used.

### [Polymerization Inhibitor]

The composition may contain a polymerization inhibitor.

As the polymerization inhibitor, known polymerization inhibitors can be used without particular limitation. Examples of the polymerization inhibitor include a phenol-based polymerization inhibitor (for example, p-methoxyphenol, 2,5-di-tert-butyl-4-methylphenol, 2,6-di-tert-butyl-4-methylphenol, 4,4'-thiobis(3-methyl-6-t-butylphenol), 2,2'-methylenebis(4-methyl-6-t-butylphenol), 4-methoxynaphthol, or the like); a hydroquinone-based polymerization inhibitor (for example, hydroquinone, 2,6-di-tert-butyl hydroquinone, or the like); a quinone-based polymerization inhibitor (for example, benzoquinone or the like); a free radical-based polymerization inhibitor (for example, a 2,2,6,6-tetramethylpiperidine 1-oxyl free radical, a 4-hydroxy-2,2,6,6-tetramethylpiperidine 1-oxyl free radical, or the like); a nitrobenzene-based polymerization inhibitor (for example, nitrobenzene, 4-nitrotoluene, or the like); a phenothiazine-based polymerization inhibitor (for example, phenothiazine, 2-methoxyphenothiazine, or the like); and the like.

Among these, a phenol-based polymerization inhibitor or a free radical-based polymerization inhibitor is preferable.

The effect of the polymerization inhibitor is marked in a case where the polymerization inhibitor is used together with a resin containing a curable group.

The content of the polymerization inhibitor in the composition is not particularly limited. The content of the polymerization inhibitor with respect to the total mass of the composition is preferably 0.0001% to 0.5% by mass, more preferably 0.0001% to 0.2% by mass, and even more preferably 0.0001% to 0.05% by mass.

The content of the polymerization inhibitor with respect to the total solid content of the composition is preferably 0.0001% to 0.5% by mass, more preferably 0.0001% to 0.2% by mass, and even more preferably 0.0001% to 0.05% by mass.

The ratio of the content of the polymerization inhibitor to the content of the polymerizable compound (particularly, the compound containing a group containing an ethylenically unsaturated bond) in the composition (content of polymerization inhibitor/content of polymerizable compound (mass ratio)) is preferably more than 0.0005, more preferably 0.0006 to 0.02, and even more preferably 0.0006 to 0.005.

### [Surfactant]

The composition may contain a surfactant. The surfactant contributes to the improvement of the coating properties of the composition.

In a case where the composition contains a surfactant, the content of the surfactant with respect to the total mass of the composition is preferably 0.001% to 2.0% by mass, more preferably 0.005% to 0.5% by mass, and even more preferably 0.01% to 0.1% by mass.

The content of the surfactant with respect to the total solid content of the composition is preferably 0.001% to 2.0% by mass, more preferably 0.005% to 0.5% by mass, and even more preferably 0.01% to 0.1% by mass.

Examples of the surfactant include a fluorine-based surfactant, a nonionic surfactant, a cationic surfactant, an anionic surfactant, a silicone-based surfactant, and the like.

For example, in a case where the composition contains a fluorine-based surfactant, the liquid properties (particularly, fluidity) of the composition are further improved. That is, in a case where a film is formed using the composition containing a fluorine-based surfactant, the interfacial tension between the surface to be coated and the coating liquid is reduced, and the wettability with respect to the surface to be coated is improved, which improves the coating properties with respect to the surface to be coated. Therefore, it is effective to use the composition containing a fluorine-based surfactant, because then a film having a uniform thickness with small thickness unevenness is more suitably formed even in a case where a thin film of about several µm is formed using a small amount of liquid.

The fluorine content in the fluorine-based surfactant is preferably 3% to 40% by mass, more preferably 5% to 30% by mass, and even more preferably 7% to 25% by mass. The fluorine-based surfactant with a fluorine content in this range is effective for achieving thickness uniformity of a coating film and/or saving liquid, and has excellent solubility in the composition.

Examples of the fluorine-based surfactant include the surfactants described in paragraphs "0060" to "0064" of JP2014-041318A (paragraphs "0060" to "0064" of WO2014/017669A corresponding to JP2014-041318A) and the like, the surfactants described in paragraphs "0117" to "0132" of JP2011-132503A, and the surfactant described JP2020-008634A. What are described in these documents are incorporated into the present specification. Examples of commercially available fluorine-based surfactants include MEGAFACE F-171, F-172, F-173, F-176, F-177, F-141, F-142, F-143, F-144., F-437, F-475, F-477, F-479, F-482, F-554, F-555-A, F-556, F-557, F-558, F-559, F-560, F-561, F-565, F-563, F-568, F-575, F-780, EXP, MFS-330, R-41, R-41-LM, R-01, R-40, R-40-LM, R-43, RS-43, TF-1956, RS-90, R-94, RS-72-K, and DS-21 (all of these are manufactured by DIC Corporation), FLUORAD FC430, FC431, and FC171 (all of these are manufactured by Sumitomo 3M Ltd.); SURFLON S-382, SC-101, SC-103, SC-104, SC-105, SC-1068, SC-381, SC-383, S-393, and KH-40 (all of these are manufactured by AGC Inc.), PolyFox PF636, PF656, PF6320, PF6520, and PF7002 (all of these are manufactured by OMNOVA Solutions), FTERGENT 710FM, 610FM, 601AD, 601ADH2, 602A, 215M, and 245F (all of these are manufactured by NEOS COMPANY LIMITED), and the like.

A block polymer can also be used as the fluorine-based surfactant, and specific examples thereof include the compounds described in JP2011-089090A.

Examples of the silicone-based surfactant include KF-6000, KF-6001, KF-6002, KF-6003, and KF-6007 (manufactured by Shin-Etsu Chemical Co., Ltd.)

From the viewpoint of environmental regulation, sometimes the use of perfluoroalkyl sulfonic acid and a salt thereof, and perfluoroalkyl carboxylic acid and a salt thereof is restricted.

In a case where the content of the above compounds in the composition is to be reduced, the content of the perfluoroalkyl sulfonic acid (particularly, perfluoroalkyl sulfonic acid having a perfluoroalkyl group with a carbon number of 6 to 8) and a salt thereof, and the perfluoroalkyl carboxylic acid (particularly, perfluoroalkyl carboxylic acid having a perfluoroalkyl group with a carbon number of 6 to 8) and a salt thereof with respect to the total solid content of the composition is preferably 0.01 to 1,000 ppb, more preferably 0.05 to 500 ppb, and even more preferably 0.1 to 300 ppb.

The composition may substantially not contain the perfluoroalkyl sulfonic acid and a salt thereof and the perfluoroalkyl carboxylic acid and a salt thereof. For example, a compound that can substitute for perfluoroalkyl sulfonic acid and a salt thereof and a compound that can substitute for perfluoroalkyl carboxylic acid and a salt thereof may be used such that the composition substantially does not contain perfluoroalkyl sulfonic acid and a salt thereof and perfluoroalkyl carboxylic acid and a salt thereof. Examples of the compound that can substitute for the regulated compound include compounds excluded from the regulation target due to the difference in the carbon number of the perfluoroalkyl group. Here, what are described above do not prevent the use of the perfluoroalkyl sulfonic acid and a salt thereof and the perfluoroalkyl carboxylic acid and a salt thereof. The composition may contain the perfluoroalkyl sulfonic acid and a salt thereof and the perfluoroalkyl carboxylic acid and a salt thereof, within the maximum allowable range.

### [Solvent]

The composition may contain a solvent.

Examples of the solvent include water and an organic solvent. As the solvent, an organic solvent is preferable.

In view of coating properties, the boiling point of the solvent is preferably 100°C to 400°C, more preferably 150°C to 300°C, and even more preferably 170°C to 250°C. In the present specification, unless otherwise specified, the boiling point means a standard boiling point.

Examples of the organic solvent include acetone, methyl ethyl ketone, cyclohexane, ethyl acetate, ethylene dichloride, tetrahydrofuran, toluene, ethylene glycol monomethyl ether, ethylene glycol monoethyl ether, ethylene glycol dimethyl ether, propylene glycol monomethyl ether, propylene glycol monoethyl ether, acetylacetone, cyclohexanone, cyclopentanone, diacetone alcohol, ethylene glycol monomethyl ether acetate, ethylene glycol ethyl ether acetate, ethylene glycol monoisopropyl ether, ethylene glycol monobutyl ether acetate, 1,4-butanedioldiacetate, 3-methoxypropanol, methoxy methoxyethanol, diethylene glycol monomethyl ether, diethylene glycol monoethyl ether, diethylene glycol dimethyl ether, diethylene glycol diethyl ether, propylene glycol monomethyl ether acetate, propylene glycol monoethyl ether acetate, 3-methoxypropyl acetate, N,N-dimethylformamide, dimethyl sulfoxide, γ-butyrolactone, ethyl acetate, butyl acetate, methyl lactate, N-methyl-2-pyrrolidone, ethyl lactate, and the like. However, the organic solvent is not limited to these.

In a case where the composition contains a solvent, in view of further improving the effects of the present invention, the content of the solvent with respect to the total mass of the composition is preferably 1% to 25% by mass, more preferably 1% to 15% by mass, and even more preferably 1% or more and less than 12% by mass.

It is also preferable that the composition substantially do not contain a solvent. For the composition, "substantially do not contain a solvent" mean that the content of the solvent with respect to the total mass of the composition is less than 1% by mass. For example, the content of the solvent is preferably 0% by mass or more and less than 1% by mass, more preferably 0% to 0.5% by mass, and even more preferably 0% to 0.1% by mass.

The concentration of solid contents of the composition is preferably 20% to 100% by mass, more preferably 40% to 100% by mass, and even more preferably 75% to 100% by mass.

### [Other optional components]

The composition may further contain other optional components in addition to the aforementioned components. Examples thereof include magnetic particles other than the specific magnetic particles, a sensitizer, a co-sensitizer, a crosslinking agent (curing agent), a thermosetting accelerator, a plasticizer, a diluent, an oil sensitizing agent, a rubber component, and the like. As necessary, known additives, such as an adhesion facilitator and other aids (for example, an antifoaming agent, a flame retardant, a leveling agent, a peeling accelerator, an antioxidant, a fragrance, a surface tension adjuster, a chain transfer agent, and the like) may be further added to a substrate surface.

### [Example of suitable aspects of composition]

One of the examples of suitable aspects of the composition include a composition containing the specific magnetic particles, a rheology control agent, and a curable component that is cured by light or heat. This composition is preferably a composition containing the specific magnetic particles, a rheology control agent, and a polymerizable compound, and more preferably a composition containing the specific magnetic particles, a rheology control agent, and a compound containing one or more epoxy groups and one or more oxetanyl groups.

In a case where the composition contains a curable component that is cured by light, it is preferable that the composition further contain a photopolymerization initiator. In a case where the composition contains a curable component that is cured by heat, the composition may further contain a thermal polymerization initiator. In a case where the composition contains a compound containing one or more epoxy groups and one or more oxetanyl groups, the composition may contain a curing accelerator.

### [Physical properties of composition]

In view of further improving sedimentation stability of the specific magnetic particles, the viscosity of the composition at 23°C and a shear rate of 0.1 (1/s) is preferably 1 to 1,000,000 Pa·s, more preferably 10 to 50,000 Pa·s, and even more preferably 50 to 10,000 Pa s.

In view of further improving sedimentation stability of the specific magnetic particles, the viscosity of the composition at 23°C and a shear rate of 1,000 (1/s) is preferably 100 Pa·s or less, more preferably 50 Pa·s or less, and even more preferably 10 Pa·s or less. The lower limit of the viscosity at a shear rate of 1,000 (1/s) is preferably 0.001 Pa s or more.

The viscosity of the composition at 23°C is obtained by measuring viscosity at 23°C by using MCR-102 (manufactured by Anton Paar GmbH) while increasing the shear rate from 0.1/s to 1,000/s.

### [Manufacturing method of composition]

The composition can be prepared by mixing together the components described above by a known mixing method (for example, a mixing method using a stirrer, a homogenizer, a high-pressure emulsifier, a wet pulverizer, a wet disperser, or the like).

In preparing the composition according to the aspect of the present invention, the components may be mixed together at once, or the components may be dissolved or dispersed one by one in a solvent and then sequentially mixed together. Furthermore, the order of adding components and working conditions at the time of mixing are not particularly limited. For example, in a case where two or more kinds of other resins are used, the resins may be mixed together at once, or each kind of resin may be mixed in batches.

### [Example of suitable form of composition]

One of the examples of suitable forms of the composition according to the embodiment of the present invention (composition A) is a composition (hereinafter, also called "composition B") containing magnetic particles that contain 70% to 90% by mass of Fe atoms, have a diffraction peak which has a half-width of 0.2° to 3° and appears at 2θ in a range of 42° to 48° in an X-ray diffraction pattern obtained by X-ray diffraction analysis, have an average particle diameter of 2 to 30 µm, and have an aspect ratio less than 8, and a rheology control agent.

### [Magnetic particle-containing film]

The magnetic particle-containing film according to an embodiment of the present invention is formed of the aforementioned composition according to the embodiment of the present invention.

In view of further improving magnetic permeability, the film thickness of the magnetic particle-containing film is preferably 1 to 10,000 µm, more preferably 10 to 1,000 µm, and even more preferably 15 to 800 µm.

The magnetic particle-containing film is suitably used as electronic components such as an antenna and an inductor installed in an electronic communication device and the like.

### [Manufacturing method of magnetic particle-containing film]

The magnetic particle-containing film according to the embodiment of the present invention is obtained, for example, by curing the aforementioned composition.

The manufacturing method of the magnetic particle-containing film is not particularly limited, but preferably includes the following steps.
- Composition layer forming step
- Curing step

### <Composition layer forming step>

In the composition layer forming step, the composition is applied to a substrate (support) or the like such that a layer of the composition (composition layer) is formed. As the substrate, for example, a wiring board having an antenna portion or an inductor portion and the like can be used.

As a method for applying the composition to the substrate, various coating methods such as a slit coating method, an inkjet method, a spin coating method, a cast coating method, a roll coating method, and a screen printing method can be used. The film thickness of the composition layer is preferably 1 to 10,000 µm, more preferably 10 to 1,000 µm, and even more preferably 15 to 800 µm. The composition layer applied to the substrate may be heated (pre-baked). The pre-baking is performed, for example, using a hot plate, an oven, or the like at a temperature of 50°C to 140°C for 10 to 1,800 seconds. Particularly, it is preferable to perform pre-baking in a case where the composition contains a solvent.

### <Curing step>

The curing step is not particularly limited as long as the composition layer can be cured, and examples thereof include a heating treatment of heating the composition layer, an exposure treatment of irradiating the composition layer with an actinic ray or radiation, and the like.

In a case where the heating treatment is performed, for example, the heating treatment can be performed continuously or in batch by using heating means such as a hot plate, a convection oven (hot air circulation-type dryer), or a high-frequency heater.

The heating temperature during the heating treatment is preferably 120°C to 260°C, and more preferably 150°C to 240°C. The heating time is not particularly limited, but is preferably 10 to 1,800 seconds.

Note that pre-baking in the composition layer forming step may serve as the heating treatment in the curing step.

In a case where the exposure treatment is performed, the method of irradiating the composition layer with an actinic ray or radiation is not particularly limited. It is preferable to irradiate the composition layer through a photomask having a patterned opening portion.

The exposure is preferably performed by irradiation with radiation. As the radiation that can be used for exposure, an ultraviolet ray such as g-line, h-line, or i-line is preferable, and a high-pressure mercury lamp is preferable as a light source. The irradiation intensity is preferably 5 to 1,500 mJ/cm², and more preferably 10 to 1,000 mJ/cm².

In a case where the composition contains a thermal polymerization initiator, the composition layer may be heated in the above exposure treatment. The heating temperature is not particularly limited, but is preferably 80°C to 250°C. The heating time is not particularly limited, but is preferably 30 to 300 seconds.

In a case where the composition layer is heated in the exposure treatment, the heating may serve as a post-heating step which will be described later. In other words, in a case where the composition layer is heated in the exposure treatment, the manufacturing method of the magnetic particle-containing film may not include a post-heating step.

### <Development step>

In a case where the exposure treatment is performed in the curing step, the manufacturing method may further include a development step.

The development step is a step of developing the exposed composition layer to form a magnetic particle-containing film. By this step, the composition layer in a portion not being irradiated with light in the exposure treatment is eluted, and only the photo-cured portion remains. In this way, a patterned magnetic particle-containing film is obtained.

Although the type of developer used in the development step is not particularly limited, it is desirable to use an alkali developer that does not damage the circuit or the like.

The development temperature is, for example, 20°C to 30°C.

The development time is, for example, 20 to 90 seconds. In recent years, in order to more thoroughly remove residues, sometimes the development has been performed for 120 to 180 seconds. Furthermore, in order to further improve the residue removability, sometimes a step of shaking off the developer every 60 seconds and supplying a new developer is repeated several times.

As the alkali developer, an alkaline aqueous solution is preferable which is prepared by dissolving an alkaline compound in water at a concentration of 0.001% to 10% by mass (preferably 0.01% to 5% by mass).

Examples of the alkaline compound include sodium hydroxide, potassium hydroxide, sodium carbonate, sodium silicate, sodium metasilicate, aqueous ammonia, ethylamine, diethylamine, dimethylethanolamine, tetramethylammonium hydroxide, tetraethylammonium hydroxide, tetrapropylammonium hydroxide, tetrabutylammonium hydroxide, benzyltrimethylammonium hydroxide, choline, pyrrole, piperidine, 1,8-diazabicyclo[5.4.0]-7-undecene, and the like (among these, an organic alkali is preferable).

In a case where an alkali developer is used, generally, a rinsing treatment using water is performed after development.

### <Post-Baking>

In a case where the exposure treatment is performed in the curing step, it is preferable to perform the heating treatment (post-baking) after the curing step. The post-baking is a heating treatment for completion of curing. In a case where the development step is performed, it is preferable to perform the post-baking after the development step. The heating temperature is preferably 240°C or lower, and more preferably 220°C or lower. The lower limit of the heating temperature is not particularly limited. However, considering an efficient and effective treatment, the heating temperature is preferably 50°C or higher, and more preferably 100°C or higher. The heating time is not particularly limited, but is preferably 10 to 1,800 seconds.

The post-baking can be performed continuously or in batch by using heating means such as a hot plate, a convection oven (hot air circulation-type dryer), or a high-frequency heater.

It is preferable that the aforementioned post-baking be performed in an atmosphere with a low oxygen concentration. The oxygen concentration is preferably 19% by volume or less, more preferably 15% by volume or less, even more preferably 10% by volume or less, particularly preferably 7% by volume or less, and most preferably 3% by volume or less. The lower limit of the oxygen concentration is not particularly limited, but is practically 10 ppm by volume or more.

Instead of post-baking by heating described above, ultraviolet (UV) irradiation may be performed to complete curing.

In this case, it is preferable that the composition further contain a UV curing agent. The UV curing agent is preferably a UV curing agent that can be cured at a wavelength shorter than 365 nm, which is the exposure wavelength of the polymerization initiator added for the lithography process by ordinary i-line exposure. Examples of the UV curing agent include Ciba IRGACURE 2959 (trade name). In a case where UV irradiation is performed, it is preferable that the composition layer be a material that is cured at a wavelength of 340 nm or less. The lower limit of the wavelength is not particularly limited, but is 220 nm or more in general. The exposure amount of UV irradiation is preferably 100 to 5,000 mJ, more preferably 300 to 4,000 mJ, and even more preferably 800 to 3,500 mJ. In order to more effectively cure the composition layer at a low temperature, it is preferable that this UV curing step be performed after the exposure treatment. As the exposure light source, it is preferable to use an ozoneless mercury lamp.

### [Electronic component]

The electronic component according to an embodiment of the present invention includes the aforementioned magnetic particle-containing film according to the embodiment of the present invention. That is, the electronic component according to the embodiment of the present invention may include the magnetic particle-containing film as a part of the component. Examples of electronic component include an inductor and an antenna. As the electronic component, an electronic component having a known structure can be used.

### Examples

Hereinafter, the present invention will be more specifically described based on examples. The materials, amounts and proportions of the materials used, details and procedures of treatments, and the like described in the following examples can be appropriately changed as long as the gist of the present invention is maintained. Therefore, the scope of the present invention is not limited to the following specific examples.

In the following description, unless otherwise specified, "%" means "% by mass", and "parts" means "parts by mass".

### [Various components used for preparing composition]

To make the composition, the components described in Table 1 were prepared. The components described in Table 1 are summarized below.

### [Magnetic particles]

As the magnetic particles, P-1 to P-4 and CP-1 to CP-5 shown below were used.

P-2 to P-4 and CP-1 to CP-2 were prepared by performing a predetermined heat treatment on Fe group amorphous. In addition, the aspect ratio was adjusted by a mechanochemical treatment using a beads mill.
· P-1: trade name "KUAMET NC1" (manufactured by Epson Atmix Corporation) "Fe nanocrystalline alloy, crystalline (having a crystal structure derived from Fe), Fe atom content: 83% by mass, D50: 23 µm, aspect ratio: 1 to 2, concentration of solid contents: 100% by mass"
· P-2: Fe nanocrystalline alloy, crystalline (having a crystal structure derived from Fe), Fe atom content: 83% by mass, D50: 3 µm, aspect ratio: 1 to 2, concentration of solid contents: 100% by mass"
·P-3: Fe nanocrystalline alloy, crystalline (having a crystal structure derived from Fe), Fe atom content: 83% by mass, D50: 30 µm, aspect ratio: 1 to 2, concentration of solid contents: 100% by mass"
· P-4: Fe nanocrystalline alloy, crystalline (having a crystal structure derived from Fe), Fe atom content: 83% by mass, D50: 28 µm, aspect ratio: 7 or more and less than 8, concentration of solid contents: 100% by mass"
· CP-1: Fe nanocrystalline alloy, crystalline (having a crystal structure derived from Fe), Fe atom content: 83% by mass, D50: 35 µm, aspect ratio: 1 to 2, concentration of solid contents: 100% by mass"
· CP-2: Fe nanocrystalline alloy, crystalline (having a crystal structure derived from Fe), Fe atom content: 83% by mass, D50: 28 µm, aspect ratio: 8 to 9, concentration of solid contents: 100% by mass"
· CP-3: trade name "AW2-08 PF-3F" (manufactured by Epson Atmix Corporation) "Fe group amorphous, noncrystalline (devoid of a crystal structure derived from Fe), Fe atom content: 87% by mass, D50: 3 µm, aspect ratio: 1 to 2, concentration of solid contents: 100% by mass"
· CP-4: trade name "EA-SMP-10 PF-5F" (manufactured by Epson Atmix Corporation) "FeSiCr, crystalline (having a crystal structure derived from Fe), Fe atom content: 92% by mass, D50: 4 µm, aspect ratio: 1 to 2, concentration of solid contents: 100% by mass"
· CP-5: trade name "JRM35G" (manufactured by Japan Metals & Chemicals Co., Ltd.) "Ni-Zn ferrite, crystalline (having a crystal structure derived from Fe), Fe atom content: < 47% by mass, D50: 33 µm, aspect ratio: 1 to 2, concentration of solid contents: 100% by mass"

### [Rheology control agent and other resins]

· D-1: trade name "BYK-P105" (manufactured by BYK-Chemie GmbH.), "polymer of low-molecular-weight unsaturated carboxylic acid, concentration of solid contents: 100% by mass"
· D-2: trade name "ANTI-TERRA-204" (manufactured by BYK-Chemie GmbH.), "solution of polyaminoamide polycarboxylate, concentration of solid contents 52% by mass"
· D-3: trade name "Talen VA705B" (manufactured by Kyoeisha Chemical Co., Ltd.), "higher fatty acid amide, concentration of solid contents: 100% by mass"
· D-4: trade name "FLOWNON RCM-230AF" (manufactured by Kyoeisha Chemical Co., Ltd.), "solution of higher fatty acid amide, concentration of solid contents 10% by mass"
· D-5: phenylphosphonic acid (manufactured by Nissan Chemical Corporation) "concentration of solid contents 100% by mass"

D-1 and D-3 are rheology control agents, and D-2 and D-4 are solutions containing a rheology control agent (solid content).
D-5 does not correspond to a rheology control agent.

### [Polymerizable Compound]

· M-1: CELLOXIDE 2021P (manufactured by Daicel Corporation), "3',4'-epoxycyclohexylmethyl-3,4-epoxycyclohexane carboxylate, concentration of solid contents 100% by mass"
· M-2: DENACOL EX-411 (manufactured by Nagase ChemteX Corporation.), "pentaerythritol polyglycidyl ether, concentration of solid contents: 100% by mass"
· M-3: KAYARAD RP-1040 (manufactured by Nippon Kayaku Co., Ltd.), "the following compound, concentration of solid contents 100% by mass" $a + b = 4 , \overline{n} = 4$
· M-4: A-TMMT (manufactured by TOAGOSEI CO., LTD.), "pentaerythritol tetraacrylate, concentration of solid contents 100% by mass"

### [Additive]

· A-1: triphenylphosphine (manufactured by TOKYO CHEMICAL INDUSTRY CO., LTD.), "concentration of solid contents: 100% by mass, curing accelerator"
· A-2: HISHICOLIN PX-4MP (manufactured by Nippon Chemical Industrial CO., LTD.), "concentration of solid contents: 100% by mass, methyltributylphosphonium dimethylphosphate, curing accelerator"
A-3: IRGACURE-OXE03 (manufactured by BASF SE) "concentration of solid contents: 100% by mass, oxime ester-based photopolymerization initiator"
A-4: Omnirad-369 (manufactured by IGM Resins B.V) "concentration of solid contents: 100% by mass, α-aminoalkylphenone-based photopolymerization initiator"
· Sur-1: MEGAFACE F-781F (manufactured by DIC Corporation), "concentration of solid contents: 100% by mass, fluorine-based surfactant"
·Sur-2: KF-6001 (manufactured by Shin-Etsu Chemical Co., Ltd.) "concentration of solid contents: 100% by mass, silicone-based surfactant, polydimethylsiloxane modified with carbinol on both terminals"

### [Solvent]

·S-1; propylene glycol monomethyl ether acetate (PGMEA) (manufactured by Tokyo Chemical Industry Co., Ltd.)
·S-2: 1,4-butanedioldiacetate (1,4-BDDA) (manufactured by Daicel Corporation)

### [Preparation of compositions of examples and comparative examples]

The components shown in Table 1 except for solvents were mixed together such that the compositional ratio (based on mass) shown in Table 1 was achieved, and the mixture was put in an airtight container made of polytetrafluoroethylene (PTFE). Thereafter, solvents were added thereto such that the compositional ratio (based on mass) shown in Table 1 was achieved, and the container was then sealed, followed by dispersion for 2 hours at 50 G by using RAM (low-frequency resonance acoustic mixer) manufactured by Resodyn Acoustic Mixers, Inc., thereby preparing compositions of examples and comparative examples.

### [Evaluation]

### [Magnetic permeability]

By using an applicator, a Si wafer having a thickness of 100 µm was coated with each of the compositions of examples and comparative examples such that a film having a thickness of 100 µm was formed. In this way, a coating film was formed.

Then, in a case where the composition with which the wafer was coated did not contain a photopolymerization initiator, the obtained coating film was dried by heating under drying conditions of 100°C for 10 minutes, and then heated at 230°C for 10 minutes, thereby preparing a substrate with a cured film. In a case where the composition with which the wafer was coated contained a photopolymerization initiator, the coating film was subjected to an exposure treatment with a proximity exposure machine under the conditions of 1,000 mJ/cm² and heated at 230°C for 10 minutes, thereby preparing a substrate with a cured film.

Thereafter, each of the obtained substrates with a cured film was cut into pieces having a size of 1 cm × 2.8 cm, thereby preparing a sample substrate for measurement.

Subsequently, by using PER-01 (manufactured by KEYCOM Corp., high-frequency magnetic permeability measuring device), for the cured film in the obtained sample substrate for measurement, the magnetic permeability was measured at 50 MHz to obtain a specific magnetic permeability µ' of the film.

Based on the obtained value of specific magnetic permeability µ', magnetic permeability was evaluated according to the following evaluation standard. For practical use, a sample graded "B" or higher is preferable.

### (Evaluation standard)

"A": 10 ≤ µ'
"B": 5 ≤ µ' < 10
"C": µ' < 5

### [Acid resistance]

The sample substrate for measurement prepared in the evaluation of magnetic permeability described above was immersed in 10% HClaq. for 30 minutes. Then, for the cured film in the substrate, magnetic permeability was measured at 50 MHz by using PER-01 (manufactured by KEYCOM Corp., high-frequency magnetic permeability measuring device) to obtain a specific magnetic permeability µ'of the film.

Subsequently, a rate of change Δµ' (%) before and after immersion was calculated by the following Equation (1). $Rate a change Δ μ ′ \left(%\right) = \left\{\begin{matrix}\left|\begin{matrix}specific magnetic permeability μ ′ after immersion - \\ specific magnetic permeability μ ′ before immersion\end{matrix}\right| / specific magnetic permeability μ ′ before \\ immersion\end{matrix}\right\} \times 100$

Based on the obtained value of rate of change Δµ', magnetic permeability was evaluated according to the following evaluation standard. For practical use, a sample graded "B" or higher is preferable.

### (Evaluation standard)

"A": Δµ' < 3%
"B": 3% <_ Δµ' < 10%
C: 10% < Δµ'

### [Sedimentation stability]

3 mL of each of the compositions of examples and comparative examples was put into a transparent glass container (cylindrical container having a diameter of 23 mm and a height of 35 mm), sealed, and left to stand at 25°C for 1 month.

Thereafter, the composition in the glass container was visually observed, and a distance d1 between the gas-liquid interface and the interface between a transparent region and an opaque region and a distance d2 between the gas-liquid interface and the bottom surface of the glass container were measured.

Subsequently, the same glass container was stirred at 3,300 rpm/min for 30 seconds by using a shaker Se-08 manufactured by TAITEC CORPORATION, and then left to stand at 25°C for 12 hours. Thereafter, the composition in the glass container was visually observed, and a distance d1' between the gas-liquid interface and the interface between a transparent region and an opaque region and a distance d2' between the gas-liquid interface and the bottom surface of the glass container were measured.

By using the distance d1, the distance d2, the distance d1', and the distance d2', sedimentation stability was evaluated based on the following standard. In a case where a sample is graded B based on the following standard, it was determined that the sample has excellent sedimentation stability. The results are shown in Table 1.

### (Evaluation standard)

"A": 0 ≤ d1/d2 ≤ 0.1 and 0 ≤ d1'/d2' ≤ 0.1 (the liquid is not completely separated over time)
"B": 0.1 < d1/d2 ≤ 0.3 and 0 ≤ d1'/d2' ≤ 0.1 (the liquid is slightly separated over time, but is restored by stirring).
"C": 0.3 < d1/d2 or 0.1 < d1'/d2' (the liquid is separated over time and is not restored even being stirred)

### [Coating suitability]

Coating suitability was evaluated based on whether or not the composition can be applied by using the applicator used in the evaluation of magnetic permeability. Specifically, the coating suitability was evaluated based on the following evaluation standard.
"A": Applicable.
"B": The composition is applicable even though the fluidity of the composition is poor.
"C": The composition has poor fluidity and is not applicable.

### The following table 1 shows the formulation of each composition and the results of evaluation tests performed on each composition.

In the following table, "Half-width of X-ray diffraction peak" means the half-width (°) of a diffraction peak which appears at 2θ in a range of 42° to 48° in an X-ray diffraction pattern obtained by X-ray diffraction analysis.

By using the following device and under the following conditions, X-ray diffraction analysis was performed on the specific magnetic particles in a powder state.
Device name: X'Pert PRO MPD (manufactured by Malvern Panalytical)
Measurement conditions: using Cu radiation source (output: 45 kV, 40 mA)
Scan conditions: scanning a range of 20° to 70° at 0.053°/step and 0.71°/min

**[Table 1]**

| | Formulation of composition | | | | | | | | | | | | Evaluation | | | | |
|---|---|---|---|---|---|---|---|---|---|---|---|---|---|---|---|---|---|
| | Magnetic particles | | Rheology control agent or other resins | | Polymerizable compound | | Additive | | Surfactant | | Solvent | | Half-width of X-ray diffraction peak (°) | Magnetic permeability µ' | Acid resistance | Sedimentation stability | Coating suitability |
| | Type | Content (% by mass) | Type | Content (% by mass) | Type | Content (% by mass) | Type | Content (% by mass) | Type | Content (% by mass) | Type | Content (% by mass) | | | | | |
| Example 1 | P-1 | 82 | D-1 | 6 | M-1 | 12 | - | - | - | - | - | - | 0.8 | A | A | A | A |
| Example 2 | P-2 | 82 | D-1 | 6 | M-1 | 12 | - | - | - | - | - | - | 0.8 | A | A | A | A |
| Example 3 | P-3 | 82 | D-1 | 6 | M-1 | 12 | - | - | - | - | - | - | 0.8 | A | A | B | A |
| Example 4 | P-4 | 82 | D-1 | 6 | M-1 | 12 | - | - | - | - | - | - | 0.8 | B | A | A | A |
| Example 5 | P-1 | 41 | D-1 | 6 | M-1 | 12 | - | - | - | - | - | - | 0.8 | A | A | A | A |
| | P-2 | 41 | | | | | | | | | | | | | | | |
| Example 6 | P-1 | 72 | D-1 | 10 | M-t | 18 | - | - | - | - | - | - | 0.8 | B | A | A | A |
| Example 7 | P-1 | 88 | D-1 | 4 | M-1 | 8 | - | - | - | - | - | - | 0.8 | A | A | A | B |
| Example 8 | P-1 | 78 | D-2 | 6 | M-1 | 10 | - | - | - | - | S-1 | 6 | 0.8 | A | A | A | A |
| Example 9 | P-1 | 80 | D-3 | 5 | M-1 | 10 | - | - | - | - | S-1 | 5 | 0.8 | A | A | A | A |
| Example 10 | P-1 | 78 | D-4 | 8 | M-1 | 10 | - | - | - | - | S-1 | 4 | 0.8 | A | A | A | A |
| Example 11 | P-1 | 82 | D-1 | 6 | M-2 | 12 | - | - | - | - | - | - | 0.8 | A | A | A | A |
| Example 12 | P-1 | 81.5 | D-1 | 6 | M-3 | 12 | A-3 | 0.5 | - | - | - | - | 0.8 | A | A | A | A |
| Example 13 | P-1 | 81.5 | D-1 | 6 | M-4 | 12 | A-3 | 0.5 | - | - | - | - | 0.8 | A | A | A | A |
| Example 14 | P-1 | 81.5 | D-1 | 6 | M-1 | 12 | A-1 | 0.5 | - | - | - | - | 0.8 | A | A | A | A |
| Example 15 | 1>-1 | 81.5 | D-1 | 6 | M-1 | 12 | A-2 | 0.5 | - | - | - | - | 0.8 | A | A | A | A |
| Example 16 | P-1 | 81.5 | D-1 | 6 | M-3 | 12 | A-4 | 0.5 | - | - | - | - | 0.8 | A | A | A | A |
| Example 17 | P-1 | 81.97 | D-1 | 6 | M-1 | 12 | - | - | Sur-1 | 0.03 | - | - | 0.8 | A | A | A | A |
| Example 18 | P-1 | 81.45 | D-1 | 6 | M-1 | 12 | - | - | Sur-2 | 0.05 | - | - | 0.8 | A | A | A | A |
| Example 19 | P-1 | 78 | D-1 | 6 | M-1 | 12 | - | - | - | - | S-1 | 4 | 0.8 | A | A | A | A |
| Example 20 | P-1 | 76 | 0.1 | 4 | M-1 | 8 | - | - | - | - | S-1 | 12 | 0.8 | A | A | B | A |
| Example 21 | P-1 | 78 | D-1 | 6 | M-1 | 12 | - | - | - | - | S-2 | 4 | 0.8 | A | A | A | A |
| Comparative Example 1 | CP-1 | 82 | D-1 | 6 | M-1 | 12 | - | - | - | - | - | - | 0.8 | A | A | C | B |
| Comparative Example 2 | CP-2 | 82 | D-1 | 6 | M-1 | 12 | - | - | - | - | - | - | 0.8 | C | A | B | A |
| Comparative Example 3 | CP-3 | 82 | D-1 | 6 | M-1 | 12 | - | - | - | - | - | - | 5.5 | A | C | A | A |
| Comparative Example 4 | CP-4 | 82 | D-1 | 6 | M-1 | 12 | - | - | - | - | - | - | 0.3 | A | C | A | A |
| Comparative Example 5 | CP-S | 82 | D-1 | 6 | M-1 | 12 | - | - | - | - | - | - | 0.5 | C | A | B | A |
| Comparative Example 6 | 1'-1 | 82 | D-5 | 6 | M-1 | 12 | - | - | - | - | - | - | 0.8 | C | A | C | A |

As is evident from the results in Table 1, with the compositions of examples, a magnetic particle-containing film having excellent magnetic permeability and excellent acid resistance can be formed. In addition, it has been revealed that the compositions of examples have excellent sedimentation stability.

Through the comparison of Examples 1 to 4, it has been confirmed that the sedimentation stability of the composition is further improved in a case where the average particle diameter (D50) of the specific magnetic particles is 28 µm or less.

Through the comparison of Examples 1 to 4, it has been confirmed that the sedimentation stability of the composition is further improved in a case where the aspect ratio of the specific magnetic particles is less than 7.

Through the comparison of Examples 1, 6, and 7, it has been confirmed that the magnetic permeability of the formed magnetic particle-containing film is further improved, in a case where the content of the specific magnetic particles is 75% by mass or more with respect to the total mass of the composition.

Through the comparison of Examples 1, 6, and 7, it has been confirmed that the coating suitability of the composition is further improved, in a case where the content of the specific magnetic particles is 85% by mass or less with respect to the total mass of the composition.

Through the comparison of Examples 1, 19, and 20, it has been confirmed that the sedimentation stability of the composition is further improved, in a case where the content of a solvent in the composition is less than 12% by mass.

In contrast, with the compositions of comparative examples, the desired effects could not be obtained.

## Claims

1. A composition comprising:
magnetic particles that contain 70% to 90% by mass of Fe atoms and have a crystal structure of Fe, an average particle diameter of 2 to 30 µm, and an aspect ratio less than 8; and
a rheology control agent.

2. A composition comprising:
magnetic particles that contain 70% to 90% by mass of Fe atoms, have a diffraction peak which has a half-width of 0.2° to 3° and appears at 2θ in a range of 42° to 48° in an X-ray diffraction pattern obtained by X-ray diffraction analysis, have an average particle diameter of 2 to 30 µm, and have an aspect ratio less than 8; and
a rheology control agent.

3. The composition according to claim 1,
wherein the magnetic particles have a diffraction peak which has a half-width of 0.2° to 3° and appears at 2θ in a range of 42° to 48° in an X-ray diffraction pattern obtained by X-ray diffraction analysis.

4. The composition according to any one of claims 1 to 3,
wherein a content of the magnetic particles is 70% to 90% by mass with respect to a total mass of the composition.

5. The composition according to any one of claims 1 to 4,
wherein the rheology control agent is one or more substances selected from the group consisting of a polycarboxylic acid, a polycarboxylic anhydride, and an amide wax.

6. The composition according to any one of claims 1 to 5, further comprising:
a curable component that is cured by light or heat.

7. The composition according to claim 6,
wherein the curable component includes a polymerizable compound.

8. The composition according to claim 7,
wherein the polymerizable compound includes a compound containing one or more epoxy groups and one or more oxetanyl groups.

9. The composition according to any one of claims 1 to 8, further comprising:
a polymerization initiator.

10. The composition according to any one of claims 1 to 9,
wherein the composition substantially does not contain a solvent, or
the composition further contains a solvent, and a content of the solvent is 1% by mass or more and less than 12% by mass with respect to a total mass of the composition.

11. A magnetic particle-containing film formed of the composition according to any one of claims 1 to 10.

12. An electronic component comprising:
the magnetic particle-containing film according to claim 11.

13. The electronic component according to claim 12,
wherein the electronic component is used as an inductor.

14. The electronic component according to claim 12,
wherein the electronic component is used as an antenna.
